



US009802250B2

(12) **United States Patent**  
**Xu**

(10) **Patent No.:** **US 9,802,250 B2**  
(45) **Date of Patent:** **\*Oct. 31, 2017**

(54) **MAGNESIUM ALLOY POWDER METAL COMPACT**

(71) Applicant: **Zhiyue Xu**, Cypress, TX (US)

(72) Inventor: **Zhiyue Xu**, Cypress, TX (US)

(73) Assignee: **BAKER HUGHES**, Houston, TX (US)

(\*) Notice: Subject to any disclaimer, the term of this patent is extended or adjusted under 35 U.S.C. 154(b) by 62 days.

This patent is subject to a terminal disclaimer.

(21) Appl. No.: **14/730,390**

(22) Filed: **Jun. 4, 2015**

(65) **Prior Publication Data**

US 2015/0266091 A1 Sep. 24, 2015

**Related U.S. Application Data**

(62) Division of application No. 13/220,824, filed on Aug. 30, 2011, now Pat. No. 9,109,269.

(51) **Int. Cl.**

*C22C 1/04* (2006.01)  
*C22C 1/10* (2006.01)  
*C22C 19/00* (2006.01)  
*B22F 1/00* (2006.01)  
*C22C 29/08* (2006.01)  
*C22C 27/04* (2006.01)  
*C22C 29/00* (2006.01)

(Continued)

(52) **U.S. Cl.**

CPC ..... *B22F 1/0003* (2013.01); *C22C 1/04* (2013.01); *C22C 23/00* (2013.01); *C22C 23/02* (2013.01); *C22C 23/04* (2013.01); *C22C 27/04* (2013.01); *C22C 29/00* (2013.01); *C22C 29/08*

(2013.01); *C22C 32/00* (2013.01); *C22C 32/001* (2013.01); *C22C 32/0015* (2013.01); *C22C 32/0052* (2013.01); *C22C 32/0068* (2013.01); *C22C 32/0084* (2013.01); *B22F 1/0044* (2013.01)

(58) **Field of Classification Search**

None  
See application file for complete search history.

(56) **References Cited**

U.S. PATENT DOCUMENTS

1,468,905 A 9/1923 Herman  
2,189,697 A 2/1940 Baker  
(Continued)

FOREIGN PATENT DOCUMENTS

CA 2783241 A1 6/2011  
CA 2783346 A1 6/2011  
(Continued)

OTHER PUBLICATIONS

“Sliding Sleeve”, Omega Completion Technology Ltd, Sep. 29, 2009, retrieved on: [www.omega-completion.com](http://www.omega-completion.com).

(Continued)

Primary Examiner — George Wyszomierski

(74) Attorney, Agent, or Firm — Cantor Colburn LLP

(57) **ABSTRACT**

A powder metal compact is disclosed. The powder metal compact includes a cellular nanomatrix comprising a nanomatrix material. The powder metal compact also includes a plurality of dispersed particles comprising a particle core material that comprises an Mg—Zr, Mg—Zn—Zr, Mg—Al—Zn—Mn, Mg—Zn—Cu—Mn or Mg—W alloy, or a combination thereof, dispersed in the cellular nanomatrix.

**28 Claims, 4 Drawing Sheets**



|      |                              |           |                      |             |         |                       |  |
|------|------------------------------|-----------|----------------------|-------------|---------|-----------------------|--|
| (51) | <b>Int. Cl.</b>              |           |                      |             |         |                       |  |
|      | <i>C22C 32/00</i>            | (2006.01) |                      | 4,554,986 A | 11/1985 | Jones                 |  |
|      | <i>C22C 23/00</i>            | (2006.01) |                      | 4,619,699 A | 10/1986 | Petkovic-Luton et al. |  |
|      | <i>C22C 23/02</i>            | (2006.01) |                      | 4,640,354 A | 2/1987  | Boisson               |  |
|      | <i>C22C 23/04</i>            | (2006.01) |                      | 4,664,962 A | 5/1987  | DesMarais, Jr.        |  |
| (56) | <b>References Cited</b>      |           |                      | 4,668,470 A | 5/1987  | Gilman et al.         |  |
|      | <b>U.S. PATENT DOCUMENTS</b> |           |                      | 4,673,549 A | 6/1987  | Ecer                  |  |
|      |                              |           |                      | 4,674,572 A | 6/1987  | Gallus                |  |
|      |                              |           |                      | 4,678,037 A | 7/1987  | Smith                 |  |
|      |                              |           |                      | 4,681,133 A | 7/1987  | Weston                |  |
|      |                              |           |                      | 4,688,641 A | 8/1987  | Knieriemen            |  |
|      |                              |           |                      | 4,690,796 A | 9/1987  | Paliwal               |  |
|      |                              |           |                      | 4,693,863 A | 9/1987  | Del Corso et al.      |  |
|      | 2,222,233 A                  | 11/1940   | Mize                 | 4,703,807 A | 11/1987 | Weston                |  |
|      | 2,225,143 A                  | 12/1940   | Baker et al.         | 4,706,753 A | 11/1987 | Ohkochi et al.        |  |
|      | 2,238,895 A                  | 4/1941    | Gage                 | 4,708,202 A | 11/1987 | Sukup et al.          |  |
|      | 2,261,292 A                  | 11/1941   | Salnikov             | 4,708,208 A | 11/1987 | Halbardier            |  |
|      | 2,294,648 A                  | 9/1942    | Ansel                | 4,709,761 A | 12/1987 | Setterberg, Jr.       |  |
|      | 2,301,624 A                  | 11/1942   | Holt                 | 4,714,116 A | 12/1987 | Brunner               |  |
|      | 2,352,993 A                  | 7/1944    | Albertson            | 4,716,964 A | 1/1988  | Erbstoesser et al.    |  |
|      | 2,394,843 A                  | 2/1946    | Cooke et al.         | 4,719,971 A | 1/1988  | Owens                 |  |
|      | 2,672,199 A                  | 3/1954    | McKenna              | 4,721,159 A | 1/1988  | Ohkochi et al.        |  |
|      | 2,753,941 A                  | 7/1956    | Hebard et al.        | 4,738,599 A | 4/1988  | Shilling              |  |
|      | 2,754,910 A                  | 7/1956    | Derrick et al.       | 4,741,973 A | 5/1988  | Condit et al.         |  |
|      | 2,933,136 A                  | 4/1960    | Ayers et al.         | 4,768,588 A | 9/1988  | Kupsa                 |  |
|      | 2,983,634 A                  | 5/1961    | Budininkas et al.    | 4,775,598 A | 10/1988 | Jaeckel               |  |
|      | 3,057,405 A                  | 10/1962   | Mallinger            | 4,784,226 A | 11/1988 | Wyatt                 |  |
|      | 3,066,391 A                  | 12/1962   | Vordahl              | 4,805,699 A | 2/1989  | Halbardier            |  |
|      | 3,106,959 A                  | 10/1963   | Huitt et al.         | 4,817,725 A | 4/1989  | Jenkins               |  |
|      | 3,142,338 A                  | 7/1964    | Brown                | 4,834,184 A | 5/1989  | Streich et al.        |  |
|      | 3,152,009 A                  | 10/1964   | Delong               | H635 H      | 6/1989  | Johnson et al.        |  |
|      | 3,196,949 A                  | 7/1965    | Thomas               | 4,850,432 A | 7/1989  | Porter et al.         |  |
|      | 3,242,988 A                  | 3/1966    | McGuire et al.       | 4,853,056 A | 8/1989  | Hoffman               |  |
|      | 3,316,748 A                  | 5/1967    | Lang et al.          | 4,869,324 A | 9/1989  | Holder                |  |
|      | 3,326,291 A                  | 6/1967    | Zandmer et al.       | 4,869,325 A | 9/1989  | Halbardier            |  |
|      | 3,343,537 A                  | 9/1967    | Graham               | 4,880,059 A | 11/1989 | Brandell et al.       |  |
|      | 3,347,317 A                  | 10/1967   | Zandemer             | 4,889,187 A | 12/1989 | Terrell et al.        |  |
|      | 3,347,714 A                  | 10/1967   | Broverman et al.     | 4,890,675 A | 1/1990  | Dew                   |  |
|      | 3,390,724 A                  | 7/1968    | Caldwell             | 4,901,794 A | 2/1990  | Baugh et al.          |  |
|      | 3,395,758 A                  | 8/1968    | Kelly et al.         | 4,909,320 A | 3/1990  | Hebert et al.         |  |
|      | 3,406,101 A                  | 10/1968   | Kilpatrick           | 4,929,415 A | 5/1990  | Okazaki               |  |
|      | 3,416,918 A                  | 12/1968   | Henry                | 4,932,474 A | 6/1990  | Schroeder, Jr. et al. |  |
|      | 3,465,181 A                  | 9/1969    | Colby et al.         | 4,938,309 A | 7/1990  | Emdy                  |  |
|      | 3,489,218 A                  | 1/1970    | Means                | 4,938,809 A | 7/1990  | Das et al.            |  |
|      | 3,513,230 A                  | 5/1970    | Rhees et al.         | 4,944,351 A | 7/1990  | Eriksen et al.        |  |
|      | 3,602,305 A                  | 8/1971    | Kisling              | 4,949,788 A | 8/1990  | Szarka et al.         |  |
|      | 3,637,446 A                  | 1/1972    | Elliott et al.       | 4,952,902 A | 8/1990  | Kawaguchi et al.      |  |
|      | 3,645,331 A                  | 2/1972    | Maurer et al.        | 4,975,412 A | 12/1990 | Okazaki et al.        |  |
|      | 3,660,049 A                  | 5/1972    | Benjamin             | 4,977,958 A | 12/1990 | Miller                |  |
|      | 3,765,484 A                  | 10/1973   | Hamby, Jr. et al.    | 4,981,177 A | 1/1991  | Carmody et al.        |  |
|      | 3,768,563 A                  | 10/1973   | Blount               | 4,986,361 A | 1/1991  | Mueller et al.        |  |
|      | 3,775,823 A                  | 12/1973   | Adolph et al.        | 4,997,622 A | 3/1991  | Regazzoni et al.      |  |
|      | 3,816,080 A                  | 6/1974    | Bomford et al.       | 5,006,044 A | 4/1991  | Walker, Sr. et al.    |  |
|      | 3,878,889 A                  | 4/1975    | Seabourn             | 5,010,955 A | 4/1991  | Springer              |  |
|      | 3,894,850 A                  | 7/1975    | Kovalchuk et al.     | 5,036,921 A | 8/1991  | Pittard et al.        |  |
|      | 3,924,677 A                  | 12/1975   | Prenner et al.       | 5,048,611 A | 9/1991  | Cochran               |  |
|      | 4,010,583 A                  | 3/1977    | Highberg             | 5,049,165 A | 9/1991  | Tselesin              |  |
|      | 4,039,717 A                  | 8/1977    | Titus                | 5,061,323 A | 10/1991 | DeLucchia             |  |
|      | 4,050,529 A                  | 9/1977    | Tagirov et al.       | 5,063,775 A | 11/1991 | Walker, Sr. et al.    |  |
|      | 4,157,732 A                  | 6/1979    | Fonner               | 5,073,207 A | 12/1991 | Faure et al.          |  |
|      | 4,248,307 A                  | 2/1981    | Silberman et al.     | 5,074,361 A | 12/1991 | Brisco et al.         |  |
|      | 4,284,137 A                  | 8/1981    | Taylor               | 5,076,869 A | 12/1991 | Bourell et al.        |  |
|      | 4,292,377 A                  | 9/1981    | Petersen et al.      | 5,084,088 A | 1/1992  | Okazaki               |  |
|      | 4,372,384 A                  | 2/1983    | Kinney               | 5,087,304 A | 2/1992  | Chang et al.          |  |
|      | 4,373,584 A                  | 2/1983    | Silberman et al.     | 5,090,480 A | 2/1992  | Pittard et al.        |  |
|      | 4,373,952 A                  | 2/1983    | Parent               | 5,095,988 A | 3/1992  | Bode                  |  |
|      | 4,374,543 A                  | 2/1983    | Richardson           | 5,103,911 A | 4/1992  | Heijnen               |  |
|      | 4,384,616 A                  | 5/1983    | Dellinger            | 5,117,915 A | 6/1992  | Mueller et al.        |  |
|      | 4,395,440 A                  | 7/1983    | Abe et al.           | 5,161,614 A | 11/1992 | Wu et al.             |  |
|      | 4,399,871 A                  | 8/1983    | Adkins et al.        | 5,171,734 A | 12/1992 | Sanjurjo et al.       |  |
|      | 4,407,368 A                  | 10/1983   | Erbstoesser          | 5,178,216 A | 1/1993  | Giroux et al.         |  |
|      | 4,422,508 A                  | 12/1983   | Rutledge, Jr. et al. | 5,181,571 A | 1/1993  | Mueller et al.        |  |
|      | 4,452,311 A                  | 6/1984    | Speegle et al.       | 5,183,631 A | 2/1993  | Kugimiya et al.       |  |
|      | 4,475,729 A                  | 10/1984   | Costigan             | 5,188,182 A | 2/1993  | Echols, III et al.    |  |
|      | 4,498,543 A                  | 2/1985    | Pye et al.           | 5,188,183 A | 2/1993  | Hopmann et al.        |  |
|      | 4,499,048 A                  | 2/1985    | Hanejko              | 5,204,055 A | 4/1993  | Sachs et al.          |  |
|      | 4,499,049 A                  | 2/1985    | Hanejko              | 5,222,867 A | 6/1993  | Walker, Sr. et al.    |  |
|      | 4,524,825 A                  | 6/1985    | Fore                 | 5,226,483 A | 7/1993  | Williamson, Jr.       |  |
|      | 4,526,840 A                  | 7/1985    | Jerabek              | 5,228,518 A | 7/1993  | Wilson et al.         |  |
|      | 4,534,414 A                  | 8/1985    | Pringle              | 5,234,055 A | 8/1993  | Cornette              |  |
|      | 4,539,175 A                  | 9/1985    | Lichti et al.        |             |         |                       |  |

(56)

## References Cited

## U.S. PATENT DOCUMENTS

|             |         |                    |              |         |                    |
|-------------|---------|--------------------|--------------|---------|--------------------|
| 5,252,365 A | 10/1993 | White              | 5,964,965 A  | 10/1999 | Schulz et al.      |
| 5,253,714 A | 10/1993 | Davis et al.       | 5,985,466 A  | 11/1999 | Atarashi et al.    |
| 5,271,468 A | 12/1993 | Streich et al.     | 5,988,287 A  | 11/1999 | Jordan, Jr. et al. |
| 5,282,509 A | 2/1994  | Schurr, III        | 5,990,051 A  | 11/1999 | Ischy et al.       |
| 5,292,478 A | 3/1994  | Scorey             | 5,992,452 A  | 11/1999 | Nelson, II         |
| 5,293,940 A | 3/1994  | Hromas et al.      | 5,992,520 A  | 11/1999 | Schultz et al.     |
| 5,304,260 A | 4/1994  | Aikawa et al.      | 6,007,314 A  | 12/1999 | Nelson, II         |
| 5,304,588 A | 4/1994  | Boysen et al.      | 6,024,915 A  | 2/2000  | Kume et al.        |
| 5,309,874 A | 5/1994  | Willermet et al.   | 6,032,735 A  | 3/2000  | Echols             |
| 5,310,000 A | 5/1994  | Arterbury et al.   | 6,036,777 A  | 3/2000  | Sachs              |
| 5,316,598 A | 5/1994  | Chang et al.       | 6,047,773 A  | 4/2000  | Zeltmann et al.    |
| 5,318,746 A | 6/1994  | Lashmore           | 6,050,340 A  | 4/2000  | Scott              |
| 5,352,522 A | 10/1994 | Kugimiya et al.    | 6,069,313 A  | 5/2000  | Kay                |
| 5,380,473 A | 1/1995  | Bogue et al.       | 6,076,600 A  | 6/2000  | Vick, Jr. et al.   |
| 5,387,380 A | 2/1995  | Cima et al.        | 6,079,496 A  | 6/2000  | Hirth              |
| 5,392,860 A | 2/1995  | Ross               | 6,085,837 A  | 7/2000  | Massinon et al.    |
| 5,394,236 A | 2/1995  | Murnick            | 6,095,247 A  | 8/2000  | Streich et al.     |
| 5,394,941 A | 3/1995  | Venditto et al.    | 6,119,783 A  | 9/2000  | Parker et al.      |
| 5,398,754 A | 3/1995  | Dinhoble           | 6,142,237 A  | 11/2000 | Christmas et al.   |
| 5,407,011 A | 4/1995  | Layton             | 6,161,622 A  | 12/2000 | Robb               |
| 5,409,555 A | 4/1995  | Fujita et al.      | 6,167,970 B1 | 1/2001  | Stout et al.       |
| 5,411,082 A | 5/1995  | Kennedy            | 6,170,583 B1 | 1/2001  | Boyce              |
| 5,417,285 A | 5/1995  | Van Buskirk et al. | 6,173,779 B1 | 1/2001  | Smith              |
| 5,425,424 A | 6/1995  | Reinhardt et al.   | 6,176,323 B1 | 1/2001  | Weirich et al.     |
| 5,427,177 A | 6/1995  | Jordan, Jr. et al. | 6,189,616 B1 | 2/2001  | Gano et al.        |
| 5,435,392 A | 7/1995  | Kennedy            | 6,189,618 B1 | 2/2001  | Beeman et al.      |
| 5,439,051 A | 8/1995  | Kennedy et al.     | 6,213,202 B1 | 4/2001  | Read, Jr.          |
| 5,454,430 A | 10/1995 | Kennedy et al.     | 6,220,350 B1 | 4/2001  | Brothers et al.    |
| 5,456,317 A | 10/1995 | Hood, III et al.   | 6,220,357 B1 | 4/2001  | Carmichael et al.  |
| 5,456,327 A | 10/1995 | Denton et al.      | 6,228,904 B1 | 5/2001  | Yadav et al.       |
| 5,464,062 A | 11/1995 | Blizzard, Jr.      | 6,237,688 B1 | 5/2001  | Burleson et al.    |
| 5,472,048 A | 12/1995 | Kennedy et al.     | 6,238,280 B1 | 5/2001  | Ritt et al.        |
| 5,474,131 A | 12/1995 | Jordan, Jr. et al. | 6,241,021 B1 | 6/2001  | Bowling            |
| 5,477,923 A | 12/1995 | Jordan, Jr. et al. | 6,248,399 B1 | 6/2001  | Hehmann            |
| 5,479,986 A | 1/1996  | Gano et al.        | 6,250,392 B1 | 6/2001  | Muth               |
| 5,506,055 A | 4/1996  | Dorfman et al.     | 6,261,432 B1 | 7/2001  | Huber et al.       |
| 5,507,439 A | 4/1996  | Story              | 6,273,187 B1 | 8/2001  | Voisin, Jr. et al. |
| 5,511,620 A | 4/1996  | Baugh et al.       | 6,276,452 B1 | 8/2001  | Davis et al.       |
| 5,524,699 A | 6/1996  | Cook               | 6,276,457 B1 | 8/2001  | Moffatt et al.     |
| 5,526,880 A | 6/1996  | Jordan, Jr. et al. | 6,279,656 B1 | 8/2001  | Sinclair et al.    |
| 5,526,881 A | 6/1996  | Martin et al.      | 6,287,445 B1 | 9/2001  | Lashmore et al.    |
| 5,529,746 A | 6/1996  | Knoss et al.       | 6,302,205 B1 | 10/2001 | Ryll               |
| 5,533,573 A | 7/1996  | Jordan, Jr. et al. | 6,315,041 B1 | 11/2001 | Carlisle et al.    |
| 5,536,485 A | 7/1996  | Kume et al.        | 6,315,050 B2 | 11/2001 | Vaynshteyn et al.  |
| 5,558,153 A | 9/1996  | Holcombe et al.    | 6,325,148 B1 | 12/2001 | Trahan et al.      |
| 5,601,924 A | 2/1997  | Beane              | 6,328,110 B1 | 12/2001 | Joubert            |
| 5,607,017 A | 3/1997  | Owens et al.       | 6,341,653 B1 | 1/2002  | Firmaniuk et al.   |
| 5,623,993 A | 4/1997  | Van Buskirk et al. | 6,341,747 B1 | 1/2002  | Schmidt et al.     |
| 5,623,994 A | 4/1997  | Robinson           | 6,349,766 B1 | 2/2002  | Bussear et al.     |
| 5,636,691 A | 6/1997  | Hendrickson et al. | 6,354,372 B1 | 3/2002  | Carisella et al.   |
| 5,641,023 A | 6/1997  | Ross et al.        | 6,354,379 B2 | 3/2002  | Miszewski et al.   |
| 5,647,444 A | 7/1997  | Williams           | 6,357,322 B1 | 3/2002  | Dolan et al.       |
| 5,665,289 A | 9/1997  | Chung et al.       | 6,357,332 B1 | 3/2002  | Vecchio            |
| 5,677,372 A | 10/1997 | Yamamoto et al.    | 6,371,206 B1 | 4/2002  | Mills              |
| 5,685,372 A | 11/1997 | Gano               | 6,372,346 B1 | 4/2002  | Toth               |
| 5,701,576 A | 12/1997 | Fujita et al.      | 6,382,244 B2 | 5/2002  | Vann               |
| 5,707,214 A | 1/1998  | Schmidt            | 6,390,195 B1 | 5/2002  | Nguyen et al.      |
| 5,709,269 A | 1/1998  | Head               | 6,390,200 B1 | 5/2002  | Allamon et al.     |
| 5,720,344 A | 2/1998  | Newman             | 6,394,180 B1 | 5/2002  | Berscheid et al.   |
| 5,728,195 A | 3/1998  | Eastman et al.     | 6,394,185 B1 | 5/2002  | Constien           |
| 5,765,639 A | 6/1998  | Muth               | 6,397,950 B1 | 6/2002  | Streich et al.     |
| 5,772,735 A | 6/1998  | Sehgal et al.      | 6,401,547 B1 | 6/2002  | Hatfield et al.    |
| 5,782,305 A | 7/1998  | Hicks              | 6,403,210 B1 | 6/2002  | Stuivinga et al.   |
| 5,797,454 A | 8/1998  | Hipp               | 6,408,946 B1 | 6/2002  | Marshall et al.    |
| 5,826,652 A | 10/1998 | Tapp               | 6,413,727 B1 | 7/2002  | Albertsen et al.   |
| 5,826,661 A | 10/1998 | Parker et al.      | 6,419,023 B1 | 7/2002  | George et al.      |
| 5,829,520 A | 11/1998 | Johnson            | 6,420,965 B1 | 10/2002 | Winzer             |
| 5,836,396 A | 11/1998 | Norman             | 6,449,097 B1 | 12/2002 | Oneal et al.       |
| 5,857,521 A | 1/1999  | Ross et al.        | 6,491,116 B2 | 12/2002 | Berscheid et al.   |
| 5,881,816 A | 3/1999  | Wright             | 6,513,598 B2 | 2/2003  | Moore et al.       |
| 5,896,819 A | 4/1999  | Turila et al.      | 6,513,600 B2 | 2/2003  | Ross               |
| 5,902,424 A | 5/1999  | Fujita et al.      | 6,540,033 B1 | 4/2003  | Sullivan et al.    |
| 5,934,372 A | 8/1999  | Muth               | 6,543,543 B2 | 4/2003  | Muth               |
| 5,941,309 A | 8/1999  | Appleton           | 6,561,275 B2 | 5/2003  | Glass et al.       |
| 5,960,881 A | 10/1999 | Allamon et al.     | 6,588,507 B2 | 7/2003  | Dusterhoff et al.  |

| (56)                  | References Cited |                      |              |         |                          |  |
|-----------------------|------------------|----------------------|--------------|---------|--------------------------|--|
| U.S. PATENT DOCUMENTS |                  |                      |              |         |                          |  |
| 6,591,915 B2          | 7/2003           | Burris et al.        | 7,234,530 B2 | 6/2007  | Gass                     |  |
| 6,601,648 B2          | 8/2003           | Ebinger              | 7,250,188 B2 | 7/2007  | Dodelet et al.           |  |
| 6,601,650 B2          | 8/2003           | Sundararajan         | 7,252,162 B2 | 8/2007  | Akinlade et al.          |  |
| 6,609,569 B2          | 8/2003           | Howlett et al.       | 7,255,172 B2 | 8/2007  | Johnson                  |  |
| 6,612,826 B1          | 9/2003           | Bauer et al.         | 7,255,178 B2 | 8/2007  | Slup et al.              |  |
| 6,613,383 B1          | 9/2003           | George et al.        | 7,264,060 B2 | 9/2007  | Wills                    |  |
| 6,619,400 B2          | 9/2003           | Brunet               | 7,267,172 B2 | 9/2007  | Hofman                   |  |
| 6,630,008 B1          | 10/2003          | Meeks, III et al.    | 7,267,178 B2 | 9/2007  | Krywitsky                |  |
| 6,634,428 B2          | 10/2003          | Krauss et al.        | 7,270,186 B2 | 9/2007  | Johnson                  |  |
| 6,662,886 B2          | 12/2003          | Russell              | 7,287,592 B2 | 10/2007 | Surjaatmadja et al.      |  |
| 6,675,889 B1          | 1/2004           | Mullins et al.       | 7,311,152 B2 | 12/2007 | Howard et al.            |  |
| 6,699,305 B2          | 3/2004           | Myrick               | 7,316,274 B2 | 1/2008  | Xu et al.                |  |
| 6,712,153 B2          | 3/2004           | Turley et al.        | 7,320,365 B2 | 1/2008  | Pia                      |  |
| 6,712,797 B1          | 3/2004           | Southern, Jr.        | 7,322,412 B2 | 1/2008  | Badalamenti et al.       |  |
| 6,713,177 B2          | 3/2004           | George et al.        | 7,322,417 B2 | 1/2008  | Rytlewski et al.         |  |
| 6,715,541 B2          | 4/2004           | Pedersen et al.      | 7,325,617 B2 | 2/2008  | Murray                   |  |
| 6,719,051 B2          | 4/2004           | Hailey, Jr. et al.   | 7,328,750 B2 | 2/2008  | Swor et al.              |  |
| 6,755,249 B2          | 6/2004           | Robison et al.       | 7,331,388 B2 | 2/2008  | Vilela et al.            |  |
| 6,769,491 B2          | 8/2004           | Zimmerman et al.     | 7,337,854 B2 | 3/2008  | Horn et al.              |  |
| 6,776,228 B2          | 8/2004           | Pedersen et al.      | 7,346,456 B2 | 3/2008  | Le Bemadjiel             |  |
| 6,779,599 B2          | 8/2004           | Mullins et al.       | 7,350,582 B2 | 4/2008  | McKeachnie et al.        |  |
| 6,799,638 B2          | 10/2004          | Butterfield, Jr.     | 7,353,879 B2 | 4/2008  | Todd et al.              |  |
| 6,810,960 B2          | 11/2004          | Pia                  | 7,360,593 B2 | 4/2008  | Constien                 |  |
| 6,817,414 B2          | 11/2004          | Lee                  | 7,360,597 B2 | 4/2008  | Blaisdell                |  |
| 6,831,044 B2          | 12/2004          | Constien             | 7,363,970 B2 | 4/2008  | Corre et al.             |  |
| 6,883,611 B2          | 4/2005           | Smith et al.         | 7,373,978 B2 | 5/2008  | Barry et al.             |  |
| 6,887,297 B2          | 5/2005           | Winter et al.        | 7,380,600 B2 | 6/2008  | Willberg et al.          |  |
| 6,896,049 B2          | 5/2005           | Moyses               | 7,384,443 B2 | 6/2008  | Mirchandani              |  |
| 6,896,061 B2          | 5/2005           | Hriscu et al.        | 7,387,158 B2 | 6/2008  | Murray et al.            |  |
| 6,899,176 B2          | 5/2005           | Hailey, Jr. et al.   | 7,387,165 B2 | 6/2008  | Lopez De Cardenas et al. |  |
| 6,899,777 B2          | 5/2005           | Vaidyanathan et al.  | 7,392,841 B2 | 7/2008  | Murray et al.            |  |
| 6,908,516 B2          | 6/2005           | Hehmann et al.       | 7,401,648 B2 | 7/2008  | Richard                  |  |
| 6,913,827 B2          | 7/2005           | George et al.        | 7,416,029 B2 | 8/2008  | Telfer et al.            |  |
| 6,926,086 B2          | 8/2005           | Patterson et al.     | 7,422,058 B2 | 9/2008  | O'Malley                 |  |
| 6,932,159 B2          | 8/2005           | Hovem                | 7,426,964 B2 | 9/2008  | Lynde et al.             |  |
| 6,939,388 B2          | 9/2005           | Angeliu              | 7,441,596 B2 | 10/2008 | Wood et al.              |  |
| 6,945,331 B2          | 9/2005           | Patel                | 7,445,049 B2 | 11/2008 | Howard et al.            |  |
| 6,951,331 B2          | 10/2005          | Haughom et al.       | 7,451,815 B2 | 11/2008 | Hailey, Jr.              |  |
| 6,959,759 B2          | 11/2005          | Doane et al.         | 7,451,817 B2 | 11/2008 | Reddy et al.             |  |
| 6,973,970 B2          | 12/2005          | Johnston et al.      | 7,461,699 B2 | 12/2008 | Richard et al.           |  |
| 6,973,973 B2          | 12/2005          | Howard et al.        | 7,464,764 B2 | 12/2008 | Xu                       |  |
| 6,983,796 B2          | 1/2006           | Bayne et al.         | 7,472,750 B2 | 1/2009  | Walker et al.            |  |
| 6,986,390 B2          | 1/2006           | Doane et al.         | 7,478,676 B2 | 1/2009  | East, Jr. et al.         |  |
| 7,013,989 B2          | 3/2006           | Hammond et al.       | 7,503,390 B2 | 3/2009  | Gomez                    |  |
| 7,013,998 B2          | 3/2006           | Ray et al.           | 7,503,399 B2 | 3/2009  | Badalamenti et al.       |  |
| 7,017,664 B2          | 3/2006           | Walker et al.        | 7,509,993 B1 | 3/2009  | Turng et al.             |  |
| 7,017,677 B2          | 3/2006           | Keshavan et al.      | 7,510,018 B2 | 3/2009  | Williamson et al.        |  |
| 7,021,389 B2          | 4/2006           | Bishop et al.        | 7,513,311 B2 | 4/2009  | Gramstad et al.          |  |
| 7,025,146 B2          | 4/2006           | King et al.          | 7,516,791 B2 | 4/2009  | Bryant et al.            |  |
| 7,028,778 B2          | 4/2006           | Krywitsky            | 7,527,103 B2 | 5/2009  | Huang et al.             |  |
| 7,044,230 B2          | 5/2006           | Starr et al.         | 7,537,825 B1 | 5/2009  | Wardle et al.            |  |
| 7,048,812 B2          | 5/2006           | Bettles et al.       | 7,552,777 B2 | 6/2009  | Murray et al.            |  |
| 7,049,272 B2          | 5/2006           | Sinclair et al.      | 7,552,779 B2 | 6/2009  | Murray                   |  |
| 7,051,805 B2          | 5/2006           | Doane et al.         | 7,559,357 B2 | 7/2009  | Clem                     |  |
| 7,059,410 B2          | 6/2006           | Bousche et al.       | 7,575,062 B2 | 8/2009  | East, Jr.                |  |
| 7,090,027 B1          | 8/2006           | Williams             | 7,579,087 B2 | 8/2009  | Maloney et al.           |  |
| 7,093,664 B2          | 8/2006           | Todd et al.          | 7,591,318 B2 | 9/2009  | Tilghman                 |  |
| 7,096,945 B2          | 8/2006           | Richards et al.      | 7,600,572 B2 | 10/2009 | Slup et al.              |  |
| 7,096,946 B2          | 8/2006           | Jasser et al.        | 7,604,049 B2 | 10/2009 | Vaidya et al.            |  |
| 7,097,807 B1          | 8/2006           | Meeks, III et al.    | 7,604,055 B2 | 10/2009 | Richard et al.           |  |
| 7,097,906 B2          | 8/2006           | Gardner              | 7,607,476 B2 | 10/2009 | Tom et al.               |  |
| 7,108,080 B2          | 9/2006           | Tessari et al.       | 7,617,871 B2 | 11/2009 | Surjaatmadja et al.      |  |
| 7,111,682 B2          | 9/2006           | Blaisdell            | 7,635,023 B2 | 12/2009 | Goldberg et al.          |  |
| 7,128,145 B2          | 10/2006          | Mickey               | 7,640,988 B2 | 1/2010  | Phi et al.               |  |
| 7,141,207 B2          | 11/2006          | Jandeska, Jr. et al. | 7,661,480 B2 | 2/2010  | Al-Anazi                 |  |
| 7,150,326 B2          | 12/2006          | Bishop et al.        | 7,661,481 B2 | 2/2010  | Todd et al.              |  |
| 7,163,066 B2          | 1/2007           | Lehr                 | 7,665,537 B2 | 2/2010  | Patel et al.             |  |
| 7,165,622 B2          | 1/2007           | Hirth et al.         | 7,686,082 B2 | 3/2010  | Marsh                    |  |
| 7,168,494 B2          | 1/2007           | Starr et al.         | 7,690,436 B2 | 4/2010  | Turley et al.            |  |
| 7,174,963 B2          | 2/2007           | Bertelsen            | 7,699,101 B2 | 4/2010  | Fripp et al.             |  |
| 7,182,135 B2          | 2/2007           | Szarka               | 7,703,510 B2 | 4/2010  | Xu                       |  |
| 7,188,559 B1          | 3/2007           | Vecchio              | 7,703,511 B2 | 4/2010  | Buyers et al.            |  |
| 7,210,527 B2          | 5/2007           | Walker et al.        | 7,708,078 B2 | 5/2010  | Stoesz                   |  |
| 7,210,533 B2          | 5/2007           | Starr et al.         | 7,709,421 B2 | 5/2010  | Jones et al.             |  |
| 7,217,311 B2          | 5/2007           | Hong et al.          | 7,712,541 B2 | 5/2010  | Loretz et al.            |  |
|                       |                  |                      | 7,723,272 B2 | 5/2010  | Crews et al.             |  |
|                       |                  |                      | 7,726,406 B2 | 6/2010  | Xu                       |  |
|                       |                  |                      | 7,735,578 B2 | 6/2010  | Loehr et al.             |  |
|                       |                  |                      | 7,743,836 B2 | 6/2010  | Cook et al.              |  |

(56)

## References Cited

## U.S. PATENT DOCUMENTS

|                |         |                     |                 |              |                      |               |
|----------------|---------|---------------------|-----------------|--------------|----------------------|---------------|
| 7,752,971 B2   | 7/2010  | Loehr               | 8,490,689 B1    | 7/2013       | McClinton et al.     |               |
| 7,757,773 B2   | 7/2010  | Rytlewski           | 8,535,604 B1    | 9/2013       | Baker et al.         |               |
| 7,762,342 B2   | 7/2010  | Richard et al.      | 8,573,295 B2    | 11/2013      | Johnson et al.       |               |
| 7,770,652 B2   | 8/2010  | Barnett             | 8,631,876 B2    | 1/2014       | Xu et al.            |               |
| 7,771,289 B2 * | 8/2010  | Palumbo .....       | A01K 87/00      | 8,956,660 B2 | 2/2015               | Launag et al. |
|                |         |                     | 473/324         | 9,079,246 B2 | 7/2015               | Xu et al.     |
| 7,775,284 B2   | 8/2010  | Richards et al.     | 9,080,098 B2    | 7/2015       | Xu et al.            |               |
| 7,775,285 B2   | 8/2010  | Surjaatmadja et al. | 9,090,955 B2 *  | 7/2015       | Xu                   |               |
| 7,775,286 B2   | 8/2010  | Duphorne            | 9,101,978 B2 *  | 8/2015       | Xu                   |               |
| 7,784,543 B2   | 8/2010  | Johnson             | 9,211,586 B1    | 12/2015      | Lavernia et al.      |               |
| 7,793,714 B2   | 9/2010  | Johnson             | 9,243,475 B2 *  | 1/2016       | Xu                   |               |
| 7,793,820 B2   | 9/2010  | Hirano et al.       | 9,260,935 B2    | 2/2016       | Murphree et al.      |               |
| 7,798,225 B2   | 9/2010  | Giroux et al.       | 2001/0040180 A1 | 11/2001      | Wittebrood et al.    |               |
| 7,798,226 B2   | 9/2010  | Themig              | 2001/0045285 A1 | 11/2001      | Russell              |               |
| 7,798,236 B2   | 9/2010  | McKeachnie et al.   | 2001/0045288 A1 | 11/2001      | Allamon et al.       |               |
| 7,806,189 B2   | 10/2010 | Frazier             | 2002/0000319 A1 | 1/2002       | Brunet               |               |
| 7,806,192 B2   | 10/2010 | Foster et al.       | 2002/007948 A1  | 1/2002       | Bayne et al.         |               |
| 7,810,553 B2   | 10/2010 | Cruickshank et al.  | 2002/0014268 A1 | 2/2002       | Vann                 |               |
| 7,810,567 B2   | 10/2010 | Daniels et al.      | 2002/0020527 A1 | 2/2002       | Kilaas et al.        |               |
| 7,819,198 B2   | 10/2010 | Birckhead et al.    | 2002/0047058 A1 | 4/2002       | Verhoff et al.       |               |
| 7,828,055 B2   | 11/2010 | Willauer et al.     | 2002/0066572 A1 | 6/2002       | Muth                 |               |
| 7,833,944 B2   | 11/2010 | Munoz et al.        | 2002/0092654 A1 | 7/2002       | Coronado et al.      |               |
| 7,849,927 B2   | 12/2010 | Herrera             | 2002/0096365 A1 | 7/2002       | Berscheidt et al.    |               |
| 7,851,016 B2   | 12/2010 | Arbab et al.        | 2002/0104616 A1 | 8/2002       | De et al.            |               |
| 7,855,168 B2   | 12/2010 | Fuller et al.       | 2002/0108756 A1 | 8/2002       | Harrall et al.       |               |
| 7,861,779 B2   | 1/2011  | Vestavik            | 2002/0136904 A1 | 9/2002       | Glass et al.         |               |
| 7,861,781 B2   | 1/2011  | D'Arcy              | 2002/0139541 A1 | 10/2002      | Sheffield et al.     |               |
| 7,874,365 B2   | 1/2011  | East, Jr. et al.    | 2002/0162661 A1 | 11/2002      | Krauss et al.        |               |
| 7,878,253 B2   | 2/2011  | Stowe et al.        | 2003/0019639 A1 | 1/2003       | Mackay               |               |
| 7,896,091 B2   | 3/2011  | Williamson et al.   | 2003/0037925 A1 | 2/2003       | Walker et al.        |               |
| 7,897,063 B1   | 3/2011  | Perry et al.        | 2003/0060374 A1 | 3/2003       | Cooke, Jr.           |               |
| 7,900,696 B1   | 3/2011  | Nish et al.         | 2003/0075326 A1 | 4/2003       | Ebinger              |               |
| 7,900,703 B2   | 3/2011  | Clark et al.        | 2003/0104147 A1 | 6/2003       | Bretschneider et al. |               |
| 7,909,096 B2   | 3/2011  | Clark et al.        | 2003/0111728 A1 | 6/2003       | Thai et al.          |               |
| 7,909,104 B2   | 3/2011  | Bjorgum             | 2003/0127013 A1 | 7/2003       | Zavitsanos et al.    |               |
| 7,909,110 B2   | 3/2011  | Sharma et al.       | 2003/0141060 A1 | 7/2003       | Hailey et al.        |               |
| 7,909,115 B2   | 3/2011  | Grove et al.        | 2003/0141061 A1 | 7/2003       | Hailey et al.        |               |
| 7,913,765 B2   | 3/2011  | Crow et al.         | 2003/0141079 A1 | 7/2003       | Doane et al.         |               |
| 7,918,275 B2   | 4/2011  | Clem                | 2003/0150614 A1 | 8/2003       | Brown et al.         |               |
| 7,931,093 B2   | 4/2011  | Foster et al.       | 2003/0155114 A1 | 8/2003       | Pedersen et al.      |               |
| 7,938,191 B2   | 5/2011  | Vaidya              | 2003/0155115 A1 | 8/2003       | Pedersen et al.      |               |
| 7,946,335 B2   | 5/2011  | Bewlaiy et al.      | 2003/0159828 A1 | 8/2003       | Howard et al.        |               |
| 7,946,340 B2   | 5/2011  | Surjaatmadja et al. | 2003/0164237 A1 | 9/2003       | Butterfield          |               |
| 7,958,940 B2   | 6/2011  | Jameson             | 2003/0183391 A1 | 10/2003      | Hriscu et al.        |               |
| 7,963,331 B2   | 6/2011  | Surjaatmadja et al. | 2003/0226668 A1 | 12/2003      | Zimmerman et al.     |               |
| 7,963,340 B2   | 6/2011  | Gramstad et al.     | 2004/0005483 A1 | 1/2004       | Lin                  |               |
| 7,963,342 B2   | 6/2011  | George              | 2004/0020832 A1 | 2/2004       | Richards et al.      |               |
| 7,980,300 B2   | 7/2011  | Roberts et al.      | 2004/0031605 A1 | 2/2004       | Mickey               |               |
| 7,987,906 B1   | 8/2011  | Troy                | 2004/0045723 A1 | 3/2004       | Slup et al.          |               |
| 7,992,763 B2   | 8/2011  | Vecchio et al.      | 2004/0055758 A1 | 3/2004       | Brezinski et al.     |               |
| 8,020,619 B1   | 9/2011  | Robertson et al.    | 2004/0058167 A1 | 3/2004       | Arbab et al.         |               |
| 8,020,620 B2   | 9/2011  | Daniels et al.      | 2004/0069502 A1 | 4/2004       | Luke                 |               |
| 8,025,104 B2   | 9/2011  | Cooke, Jr.          | 2004/0089449 A1 | 5/2004       | Walton et al.        |               |
| 8,028,767 B2   | 10/2011 | Radford et al.      | 2004/0094297 A1 | 5/2004       | Malone et al.        |               |
| 8,033,331 B2   | 10/2011 | Themig              | 2004/0154806 A1 | 8/2004       | Bode et al.          |               |
| 8,039,422 B1   | 10/2011 | Al-Zahrani          | 2004/0159428 A1 | 8/2004       | Hammond et al.       |               |
| 8,056,628 B2   | 11/2011 | Whitsitt et al.     | 2004/0159446 A1 | 8/2004       | Haugen et al.        |               |
| 8,056,638 B2   | 11/2011 | Clayton et al.      | 2004/0182583 A1 | 9/2004       | Doane et al.         |               |
| 8,109,340 B2   | 2/2012  | Doane et al.        | 2004/0216868 A1 | 11/2004      | Owen, Sr.            |               |
| 8,127,856 B1   | 3/2012  | Nish et al.         | 2004/0231845 A1 | 11/2004      | Cooke, Jr.           |               |
| 8,153,052 B2   | 4/2012  | Jackson et al.      | 2004/0251025 A1 | 12/2004      | Giroux et al.        |               |
| 8,163,060 B2   | 4/2012  | Imanishi et al.     | 2004/0256109 A1 | 12/2004      | Johnson              |               |
| 8,211,247 B2   | 7/2012  | Marya et al.        | 2004/0256157 A1 | 12/2004      | Tessari et al.       |               |
| 8,211,248 B2   | 7/2012  | Marya               | 2004/0261993 A1 | 12/2004      | Nguyen               |               |
| 8,226,740 B2   | 7/2012  | Chaumonnot et al.   | 2004/0261994 A1 | 12/2004      | Nguyen et al.        |               |
| 8,230,731 B2   | 7/2012  | Dyer et al.         | 2005/0034876 A1 | 2/2005       | Doane et al.         |               |
| 8,231,947 B2   | 7/2012  | Vaidya et al.       | 2005/0051329 A1 | 3/2005       | Blaisdell            |               |
| 8,263,178 B2   | 9/2012  | Boulos et al.       | 2005/0064247 A1 | 3/2005       | Sane et al.          |               |
| 8,276,670 B2   | 10/2012 | Patel               | 2005/0069449 A1 | 3/2005       | Jackson et al.       |               |
| 8,277,974 B2   | 10/2012 | Kumar et al.        | 2005/0074612 A1 | 4/2005       | Eklund et al.        |               |
| 8,297,364 B2   | 10/2012 | Agrawal et al.      | 2005/0098313 A1 | 5/2005       | Atkins et al.        |               |
| 8,327,931 B2   | 12/2012 | Agrawal et al.      | 2005/0102255 A1 | 5/2005       | Bultman              |               |
| 8,403,037 B2   | 3/2013  | Agrawal et al.      | 2005/0106316 A1 | 5/2005       | Rigney et al.        |               |
| 8,425,651 B2   | 4/2013  | Xu et al.           | 2005/0126334 A1 | 6/2005       | Mirchandani          |               |
| 8,459,347 B2   | 6/2013  | Stout               | 2005/0161224 A1 | 7/2005       | Leismer et al.       |               |
|                |         |                     | 2005/0165149 A1 | 7/2005       | Starr et al.         |               |
|                |         |                     | 2005/0194143 A1 | 9/2005       | Chanak et al.        |               |
|                |         |                     | 2005/0199401 A1 | 9/2005       | Xu et al.            |               |
|                |         |                     | 2005/0199401 A1 | 9/2005       | Patel et al.         |               |

(56)

## References Cited

## U.S. PATENT DOCUMENTS

|                 |         |                          |                 |         |                     |
|-----------------|---------|--------------------------|-----------------|---------|---------------------|
| 2005/0205264 A1 | 9/2005  | Starr et al.             | 2007/0299510 A1 | 12/2007 | Venkatraman et al.  |
| 2005/0205265 A1 | 9/2005  | Todd et al.              | 2008/0011473 A1 | 1/2008  | Wood et al.         |
| 2005/0205266 A1 | 9/2005  | Todd et al.              | 2008/0020923 A1 | 1/2008  | Debe et al.         |
| 2005/0235757 A1 | 10/2005 | De Jonge et al.          | 2008/0047707 A1 | 2/2008  | Boney et al.        |
| 2005/0241824 A1 | 11/2005 | Burris, II et al.        | 2008/0060810 A9 | 3/2008  | Nguyen et al.       |
| 2005/0241825 A1 | 11/2005 | Burris, II et al.        | 2008/0066923 A1 | 3/2008  | Xu                  |
| 2005/0257936 A1 | 11/2005 | Lehr                     | 2008/0066924 A1 | 3/2008  | Xu                  |
| 2005/0268746 A1 | 12/2005 | Abkowitz et al.          | 2008/0072705 A1 | 3/2008  | Chaumonnot et al.   |
| 2005/0269097 A1 | 12/2005 | Towler                   | 2008/0078553 A1 | 4/2008  | George              |
| 2005/0275143 A1 | 12/2005 | Toth                     | 2008/0081866 A1 | 4/2008  | Gong et al.         |
| 2005/0279501 A1 | 12/2005 | Surjaatmadja et al.      | 2008/0093073 A1 | 4/2008  | Bustos et al.       |
| 2006/0012087 A1 | 1/2006  | Matsuda et al.           | 2008/0099209 A1 | 5/2008  | Loretz et al.       |
| 2006/0013350 A1 | 1/2006  | Akers                    | 2008/0105438 A1 | 5/2008  | Jordan et al.       |
| 2006/0045787 A1 | 3/2006  | Jandeska et al.          | 2008/0115932 A1 | 5/2008  | Cooke               |
| 2006/0057479 A1 | 3/2006  | Niimi et al.             | 2008/0121390 A1 | 5/2008  | O'Malley et al.     |
| 2006/0081378 A1 | 4/2006  | Howard et al.            | 2008/0121436 A1 | 5/2008  | Slay et al.         |
| 2006/0102871 A1 | 5/2006  | Wang                     | 2008/0127475 A1 | 6/2008  | Griffo              |
| 2006/0108114 A1 | 5/2006  | Johnson et al.           | 2008/0135249 A1 | 6/2008  | Fripp et al.        |
| 2006/0108126 A1 | 5/2006  | Horn et al.              | 2008/0149325 A1 | 6/2008  | Crawford            |
| 2006/0110615 A1 | 5/2006  | Karim et al.             | 2008/0149345 A1 | 6/2008  | Marya et al.        |
| 2006/0116696 A1 | 6/2006  | Odermatt et al.          | 2008/0149351 A1 | 6/2008  | Marya et al.        |
| 2006/0124310 A1 | 6/2006  | Lopez De Cardenas et al. | 2008/0169105 A1 | 7/2008  | Williamson et al.   |
| 2006/0124312 A1 | 6/2006  | Rytlewski et al.         | 2008/0169130 A1 | 7/2008  | Norman et al.       |
| 2006/0131011 A1 | 6/2006  | Lynde et al.             | 2008/0179060 A1 | 7/2008  | Surjaatmadja et al. |
| 2006/0131031 A1 | 6/2006  | McKeachnie et al.        | 2008/0179104 A1 | 7/2008  | Zhang et al.        |
| 2006/0131081 A1 | 6/2006  | Mirchandani et al.       | 2008/0196801 A1 | 8/2008  | Zhao et al.         |
| 2006/0144515 A1 | 7/2006  | Tada et al.              | 2008/0202764 A1 | 8/2008  | Clayton et al.      |
| 2006/0150770 A1 | 7/2006  | Freim                    | 2008/0202814 A1 | 8/2008  | Lyons et al.        |
| 2006/0151178 A1 | 7/2006  | Howard et al.            | 2008/0210473 A1 | 9/2008  | Zhang et al.        |
| 2006/0153728 A1 | 7/2006  | Schoenung et al.         | 2008/0216383 A1 | 9/2008  | Pierick et al.      |
| 2006/0162927 A1 | 7/2006  | Walker et al.            | 2008/0223586 A1 | 9/2008  | Barnett             |
| 2006/0169453 A1 | 8/2006  | Savery et al.            | 2008/0223587 A1 | 9/2008  | Cherewyk            |
| 2006/0186602 A1 | 8/2006  | Martin et al.            | 2008/0236829 A1 | 10/2008 | Lynde               |
| 2006/0207763 A1 | 9/2006  | Hofman et al.            | 2008/0236842 A1 | 10/2008 | Bhavsar et al.      |
| 2006/0213670 A1 | 9/2006  | Bishop et al.            | 2008/0248205 A1 | 10/2008 | Blanchet et al.     |
| 2006/0231253 A1 | 10/2006 | Vilela et al.            | 2008/0248413 A1 | 10/2008 | Ishii et al.        |
| 2006/0283592 A1 | 12/2006 | Sierra et al.            | 2008/0264205 A1 | 10/2008 | Zeng et al.         |
| 2007/0017674 A1 | 1/2007  | Blaisdell                | 2008/0264594 A1 | 10/2008 | Lohmueller et al.   |
| 2007/0017675 A1 | 1/2007  | Hammami                  | 2008/0277109 A1 | 11/2008 | Vaidya              |
| 2007/0029082 A1 | 2/2007  | Giroux et al.            | 2008/0277980 A1 | 11/2008 | Koda et al.         |
| 2007/0039161 A1 | 2/2007  | Garcia                   | 2008/0282924 A1 | 11/2008 | Saenger et al.      |
| 2007/0039741 A1 | 2/2007  | Hailey                   | 2008/0296024 A1 | 12/2008 | Huang et al.        |
| 2007/0044958 A1 | 3/2007  | Rytlewski et al.         | 2008/0302538 A1 | 12/2008 | Hofman              |
| 2007/0044966 A1 | 3/2007  | Davies et al.            | 2008/0314581 A1 | 12/2008 | Brown               |
| 2007/0051521 A1 | 3/2007  | Fike et al.              | 2008/0314588 A1 | 12/2008 | Langlais et al.     |
| 2007/0053785 A1 | 3/2007  | Hetz et al.              | 2009/0038858 A1 | 2/2009  | Griffo et al.       |
| 2007/0054101 A1 | 3/2007  | Sigalas et al.           | 2009/0044946 A1 | 2/2009  | Schasteen et al.    |
| 2007/0057415 A1 | 3/2007  | Katagiri et al.          | 2009/0044949 A1 | 2/2009  | King et al.         |
| 2007/0062644 A1 | 3/2007  | Nakamura et al.          | 2009/0050334 A1 | 2/2009  | Marya et al.        |
| 2007/0074601 A1 | 4/2007  | Hong et al.              | 2009/0056934 A1 | 3/2009  | Xu                  |
| 2007/0074873 A1 | 4/2007  | McKeachnie et al.        | 2009/0065216 A1 | 3/2009  | Frazier             |
| 2007/0102199 A1 | 5/2007  | Smith et al.             | 2009/0074603 A1 | 3/2009  | Chan et al.         |
| 2007/0107899 A1 | 5/2007  | Werner et al.            | 2009/0084553 A1 | 4/2009  | Rytlewski et al.    |
| 2007/0107908 A1 | 5/2007  | Vaidya et al.            | 2009/0084556 A1 | 4/2009  | Richards et al.     |
| 2007/0108060 A1 | 5/2007  | Park                     | 2009/0084600 A1 | 4/2009  | Severance           |
| 2007/0119600 A1 | 5/2007  | Slup et al.              | 2009/0090440 A1 | 4/2009  | Kellett et al.      |
| 2007/0131912 A1 | 6/2007  | Simone et al.            | 2009/0107684 A1 | 4/2009  | Cooke, Jr.          |
| 2007/0134496 A1 | 6/2007  | Katagiri et al.          | 2009/0114381 A1 | 5/2009  | Stroobants          |
| 2007/0151009 A1 | 7/2007  | Conrad, III et al.       | 2009/0114382 A1 | 5/2009  | Grove et al.        |
| 2007/0151769 A1 | 7/2007  | Slutz et al.             | 2009/0126436 A1 | 5/2009  | Fly et al.          |
| 2007/0169935 A1 | 7/2007  | Akbar et al.             | 2009/0139720 A1 | 6/2009  | Frazier             |
| 2007/0181224 A1 | 8/2007  | Marya et al.             | 2009/0145666 A1 | 6/2009  | Radford et al.      |
| 2007/0185655 A1 | 8/2007  | Le Bemadjiel             | 2009/0151949 A1 | 6/2009  | Marya et al.        |
| 2007/0187095 A1 | 8/2007  | Walker et al.            | 2009/0152009 A1 | 6/2009  | Slay et al.         |
| 2007/0207182 A1 | 9/2007  | Weber et al.             | 2009/0155616 A1 | 6/2009  | Thamida et al.      |
| 2007/0221373 A1 | 9/2007  | Murray                   | 2009/0159289 A1 | 6/2009  | Avant et al.        |
| 2007/0221384 A1 | 9/2007  | Murray                   | 2009/0178808 A1 | 7/2009  | Williamson et al.   |
| 2007/0227745 A1 | 10/2007 | Roberts et al.           | 2009/0194273 A1 | 8/2009  | Surjaatmadja et al. |
| 2007/0259994 A1 | 11/2007 | Tour et al.              | 2009/0205841 A1 | 8/2009  | Kluge et al.        |
| 2007/0261862 A1 | 11/2007 | Murray                   | 2009/0211770 A1 | 8/2009  | Nutley et al.       |
| 2007/0272411 A1 | 11/2007 | Lopez De Cardenas et al. | 2009/0226340 A1 | 9/2009  | Marya               |
| 2007/0272413 A1 | 11/2007 | Rytlewski et al.         | 2009/0226704 A1 | 9/2009  | Kauppinen et al.    |
| 2007/0277979 A1 | 12/2007 | Todd et al.              | 2009/0242202 A1 | 10/2009 | Rispler et al.      |
| 2007/0284109 A1 | 12/2007 | East et al.              | 2009/0242208 A1 | 10/2009 | Bolding             |
| 2007/0284112 A1 | 12/2007 | Magne et al.             | 2009/0242214 A1 | 10/2009 | Foster et al.       |
|                 |         |                          | 2009/0255667 A1 | 10/2009 | Clem et al.         |
|                 |         |                          | 2009/0255684 A1 | 10/2009 | Bolding             |
|                 |         |                          | 2009/0255686 A1 | 10/2009 | Richard             |
|                 |         |                          | 2009/0260817 A1 | 10/2009 | Gambier et al.      |

| (56)                  | References Cited |                          |                 |             |                     |  |  |
|-----------------------|------------------|--------------------------|-----------------|-------------|---------------------|--|--|
| U.S. PATENT DOCUMENTS |                  |                          |                 |             |                     |  |  |
| 2009/0266548 A1       | 10/2009          | Olsen et al.             | 2011/0253387 A1 | 10/2011     | Ervin               |  |  |
| 2009/0272544 A1       | 11/2009          | Giroux et al.            | 2011/0256356 A1 | 10/2011     | Tomantschger et al. |  |  |
| 2009/0283270 A1       | 11/2009          | Langeslag                | 2011/0259610 A1 | 10/2011     | Shkurti et al.      |  |  |
| 2009/0293672 A1       | 12/2009          | Mirchandani et al.       | 2011/0277987 A1 | 11/2011     | Frazier             |  |  |
| 2009/0301730 A1       | 12/2009          | Gweily                   | 2011/0277989 A1 | 11/2011     | Frazier             |  |  |
| 2009/0305131 A1       | 12/2009          | Kumar et al.             | 2011/0284232 A1 | 11/2011     | Huang               |  |  |
| 2009/0308588 A1       | 12/2009          | Howell et al.            | 2011/0284240 A1 | 11/2011     | Chen et al.         |  |  |
| 2009/0317556 A1       | 12/2009          | Macary                   | 2011/0284243 A1 | 11/2011     | Frazier             |  |  |
| 2009/0317622 A1       | 12/2009          | Huang et al.             | 2011/0300403 A1 | 12/2011     | Vecchio et al.      |  |  |
| 2010/0003536 A1       | 1/2010           | Smith et al.             | 2011/0314881 A1 | 12/2011     | Hatcher et al.      |  |  |
| 2010/0012385 A1       | 1/2010           | Drivdahl et al.          | 2012/0024109 A1 | 2/2012      | Xu et al.           |  |  |
| 2010/0015002 A1       | 1/2010           | Barrera et al.           | 2012/0067426 A1 | 3/2012      | Soni et al.         |  |  |
| 2010/0015469 A1       | 1/2010           | Romanowski et al.        | 2012/0090839 A1 | 4/2012      | Rudic               |  |  |
| 2010/0025255 A1       | 2/2010           | Su et al.                | 2012/0103135 A1 | 5/2012      | Xu et al.           |  |  |
| 2010/0032151 A1       | 2/2010           | Duphorne et al.          | 2012/0107590 A1 | 5/2012      | Xu et al.           |  |  |
| 2010/0034857 A1       | 2/2010           | Launag et al.            | 2012/0118583 A1 | 5/2012      | Johnson et al.      |  |  |
| 2010/0038076 A1       | 2/2010           | Spray et al.             | 2012/0130470 A1 | 5/2012      | Agnew               |  |  |
| 2010/0038595 A1       | 2/2010           | Imholt et al.            | 2012/0145378 A1 | 6/2012      | Frazier et al.      |  |  |
| 2010/0040180 A1       | 2/2010           | Kim et al.               | 2012/0145389 A1 | 6/2012      | Fitzpatrick, Jr.    |  |  |
| 2010/0044041 A1       | 2/2010           | Smith et al.             | 2012/0168152 A1 | 7/2012      | Casciaro et al.     |  |  |
| 2010/0051278 A1       | 3/2010           | Mytopher et al.          | 2012/0177905 A1 | 7/2012      | Seals et al.        |  |  |
| 2010/0055491 A1       | 3/2010           | Vecchio et al.           | 2012/0205120 A1 | 8/2012      | Howell              |  |  |
| 2010/0055492 A1       | 3/2010           | Barsoum et al.           | 2012/0205872 A1 | 8/2012      | Reinhardt et al.    |  |  |
| 2010/0089583 A1       | 4/2010           | Xu et al.                | 2012/0211239 A1 | 8/2012      | Kritzler et al.     |  |  |
| 2010/0089587 A1       | 4/2010           | Stout                    | 2012/0234546 A1 | 9/2012      | Xu et al.           |  |  |
| 2010/0101803 A1       | 4/2010           | Clayton et al.           | 2012/0234547 A1 | 9/2012      | O'Malley et al.     |  |  |
| 2010/0116495 A1       | 5/2010           | Spray                    | 2012/0267101 A1 | 10/2012     | Cooke               |  |  |
| 2010/0122817 A1       | 5/2010           | Surjaatmadja et al.      | 2012/0292053 A1 | 11/2012     | Xu et al.           |  |  |
| 2010/0139930 A1       | 6/2010           | Patel et al.             | 2012/0318513 A1 | 12/2012     | Mazyar et al.       |  |  |
| 2010/0200230 A1       | 8/2010           | East, Jr. et al.         | 2013/0004847 A1 | 1/2013      | Kumar et al.        |  |  |
| 2010/0236793 A1       | 9/2010           | Bjorgum                  | 2013/0008671 A1 | 1/2013      | Booth et al.        |  |  |
| 2010/0236794 A1       | 9/2010           | Duan et al.              | 2013/0025409 A1 | 1/2013      | Xu                  |  |  |
| 2010/0243254 A1       | 9/2010           | Murphy et al.            | 2013/0029886 A1 | 1/2013      | Mazyar et al.       |  |  |
| 2010/0252273 A1       | 10/2010          | Duphorne                 | 2013/0032357 A1 | 2/2013      | Mazyar et al.       |  |  |
| 2010/0252280 A1       | 10/2010          | Swor et al.              | 2013/0048304 A1 | 2/2013      | Agrawal et al.      |  |  |
| 2010/0270031 A1       | 10/2010          | Patel                    | 2013/0048305 A1 | 2/2013      | Xu et al.           |  |  |
| 2010/0276136 A1       | 11/2010          | Evans et al.             | 2013/0052472 A1 | 2/2013      | Xu                  |  |  |
| 2010/0276159 A1       | 11/2010          | Mailand et al.           | 2013/0081814 A1 | 4/2013      | Gaudette et al.     |  |  |
| 2010/0282338 A1       | 11/2010          | Gerrard et al.           | 2013/0084643 A1 | 4/2013      | Commarie et al.     |  |  |
| 2010/0282469 A1       | 11/2010          | Richard et al.           | 2013/0105159 A1 | 5/2013      | Alvarez             |  |  |
| 2010/0294510 A1       | 11/2010          | Holmes                   | 2013/0126190 A1 | 5/2013      | Mazyar et al.       |  |  |
| 2010/0297432 A1       | 11/2010          | Sherman et al.           | 2013/0133897 A1 | 5/2013      | Baihly et al.       |  |  |
| 2010/0304182 A1*      | 12/2010          | Facchini .....           | 2013/0146144 A1 | 6/2013      | Joseph et al.       |  |  |
|                       |                  | B32B 15/013              | 2013/0146302 A1 | 6/2013      | Gaudette et al.     |  |  |
|                       |                  | 428/652                  | 2013/0168257 A1 | 7/2013      | Mazyar et al.       |  |  |
| 2010/0314105 A1       | 12/2010          | Rose                     | 2013/0186626 A1 | 7/2013      | Aitken et al.       |  |  |
| 2010/0314126 A1       | 12/2010          | Kellner                  | 2013/0240200 A1 | 9/2013      | Frazier             |  |  |
| 2010/0319427 A1       | 12/2010          | Lohbeck                  | 2013/0240203 A1 | 9/2013      | Frazier             |  |  |
| 2010/0319870 A1       | 12/2010          | Bewlay et al.            | 2013/0299185 A1 | 11/2013     | Xu et al.           |  |  |
| 2010/0326650 A1       | 12/2010          | Tran et al.              | 2013/0299192 A1 | 11/2013     | Xu et al.           |  |  |
| 2011/0005773 A1       | 1/2011           | Dusterhoff et al.        | 2013/0300066 A1 | 11/2013     | Xu et al.           |  |  |
| 2011/0036592 A1       | 2/2011           | Fay                      | 2013/0319668 A1 | 12/2013     | Tschetter et al.    |  |  |
| 2011/0048743 A1       | 3/2011           | Stafford et al.          | 2013/0327540 A1 | 12/2013     | Hamid et al.        |  |  |
| 2011/0052805 A1       | 3/2011           | Bordere et al.           | 2014/0014339 A1 | 1/2014      | O'Malley et al.     |  |  |
| 2011/0056692 A1       | 3/2011           | Lopez De Cardenas et al. | 2014/0027128 A1 | 1/2014      | Johnson et al.      |  |  |
| 2011/0056702 A1       | 3/2011           | Sharma et al.            | 2014/0060834 A1 | 3/2014      | Quintero et al.     |  |  |
| 2011/0067872 A1       | 3/2011           | Agrawal                  | 2014/0116711 A1 | 5/2014      | Tang et al.         |  |  |
| 2011/0067889 A1       | 3/2011           | Marya et al.             | 2014/0262327 A1 | 9/2014      | Xu et al.           |  |  |
| 2011/0067890 A1       | 3/2011           | Themig                   | 2014/0360728 A1 | 12/2014     | Tashiro et al.      |  |  |
| 2011/0094406 A1       | 4/2011           | Marya et al.             | 2015/0060085 A1 | 3/2015      | Xu                  |  |  |
| 2011/0100643 A1       | 5/2011           | Themig et al.            | 2015/0065401 A1 | 3/2015      | Xu et al.           |  |  |
| 2011/0127044 A1       | 6/2011           | Radford et al.           | 2016/0209391 A1 | 7/2016      | Zhang et al.        |  |  |
| 2011/0132143 A1       | 6/2011           | Xu et al.                | 2016/0258242 A1 | 9/2016      | Hayter et al.       |  |  |
| 2011/0132612 A1       | 6/2011           | Agrawal et al.           | CN              | 1076968 A   | 10/1993             |  |  |
| 2011/0132619 A1       | 6/2011           | Agrawal et al.           | CN              | 1079234 A   | 12/1993             |  |  |
| 2011/0132620 A1       | 6/2011           | Agrawal et al.           | CN              | 1255879 A   | 6/2000              |  |  |
| 2011/0132621 A1       | 6/2011           | Agrawal et al.           | CN              | 2658384 Y   | 11/2004             |  |  |
| 2011/0135530 A1       | 6/2011           | Xu et al.                | CN              | 1668545 A   | 9/2005              |  |  |
| 2011/0135805 A1       | 6/2011           | Doucet et al.            | CN              | 1882759 A1  | 12/2006             |  |  |
| 2011/0135953 A1       | 6/2011           | Xu et al.                | CN              | 101050417 A | 10/2007             |  |  |
| 2011/0136707 A1       | 6/2011           | Xu et al.                | CN              | 101351523 A | 1/2009              |  |  |
| 2011/0139465 A1       | 6/2011           | Tibbles et al.           | CN              | 101454074 A | 6/2009              |  |  |
| 2011/0147014 A1       | 6/2011           | Chen et al.              | CN              | 101457321 A | 6/2009              |  |  |
| 2011/0186306 A1       | 8/2011           | Marya et al.             | CN              | 101605963   | 12/2009             |  |  |
| 2011/0214881 A1       | 9/2011           | Newton                   | CN              | 101720378 A | 6/2010              |  |  |
| 2011/0247833 A1       | 10/2011          | Todd et al.              | EP              | 0033625 A1  | 8/1981              |  |  |

## FOREIGN PATENT DOCUMENTS

(56)

## References Cited

## FOREIGN PATENT DOCUMENTS

EP 1006258 A2 6/2000  
 EP 1174385 A2 1/2002  
 EP 1412175 A1 4/2004  
 EP 1798301 A1 8/2006  
 EP 1857570 A2 11/2007  
 FR 2782096 A1 2/2000  
 GB 912956 A 12/1962  
 GB 1046330 A 10/1966  
 GB 1280833 A 7/1972  
 GB 1357065 A 6/1974  
 JP 61067770 A 4/1986  
 JP 07-054008 A 2/1995  
 JP 08-232029 A 9/1996  
 JP 2000185725 A1 7/2000  
 JP 2002053902 A 2/2002  
 JP 2004225084 A 8/2004  
 JP 2004225765 A 8/2004  
 JP 2005076052 A 3/2005  
 JP 2009144207 A 7/2009  
 JP 2010502840 A 1/2010  
 KR 950014350 B1 11/1995  
 WO 9909227 A1 2/1999  
 WO 9947726 A1 9/1999  
 WO 03008186 A1 1/2003  
 WO 2004001087 A1 12/2003  
 WO 2004073889 A1 9/2004  
 WO 2005040068 A 5/2005  
 WO 2007044635 A 4/2007  
 WO 2007095376 A2 8/2007  
 WO 2008034042 A3 3/2008  
 WO 2008057045 A1 5/2008  
 WO 2008079485 A2 7/2008  
 WO 2008079777 A2 7/2008  
 WO 2009079745 A1 7/2009  
 WO 2010012184 A1 2/2010  
 WO 2011071902 A2 6/2011  
 WO 2011071907 A2 6/2011  
 WO 2011071910 A2 6/2011  
 WO 2011071910 A3 6/2011  
 WO 2011130063 A3 2/2012  
 WO 2012015567 A2 2/2012  
 WO 2012149007 A2 11/2012  
 WO 2012164236 A1 12/2012  
 WO 2012174101 A2 12/2012  
 WO 2013053057 A1 4/2013  
 WO 2013078031 A1 5/2013  
 WO 2014121384 A1 8/2014

## OTHER PUBLICATIONS

Ambat, et al., "Electroless Nickel-Plating on AZ91D Magnesium Alloy: Effect of Substrate Microstructure and Plating Parameters"; Surface and Coatings Technology; 179; pp. 124-134; (2004).  
 Baker Oil Tools, "Baker Oil Tools Introduces Revolutionary Sand Control Completion Technology," May 2, 2005.  
 Baker Oil Tools, "Z-Seal Metal-to-Metal Expandable Sealing Device Uses Expanding Metal in Place of Elastomers," Nov. 6, 2006.  
 Bastow, et al., "Clustering and formation of nano-precipitates in dilute aluminum and magnesium alloys", Materials Science and Engineering, 2003, C23, 757-762.  
 Bercegeay, et al., "A One-Trip Gravel Packing System"; Society of Petroleum Engineers, Offshore Technology Conference, SPE Paper No. 4771; Feb. 7-8, 1974.  
 Bybee, "One-Trip Completion System Eliminates Perforations," Completions Today, Sep. 2007, pp. 52-53.  
 Canadian Office Action for Canadian Application No. 2,783,547, dated Feb. 15, 2013, pp. 1-3.  
 Chang, et al., "Electrodeposition of Aluminum on Magnesium Alloy in Aluminum Chloride (AlC13)-1-ethyl-3-methylimidazolium chloride (EMIC) Ionic Liquid and Its Corrosion Behavior"; Electrochemistry Communications; 9; pp. 1602-1606; (2007).  
 Christoglou, et al., "Deposition of Aluminum on Magnesium by a CVD Process", Surface and Coatings Technology 184 (2004) 149-155.  
 Constantine, "Selective Production of Horizontal Openhole Completions Using ECP and Sliding Sleeve Technology." SPE Rocky Mountain Regional Meeting, May 15-18, 1999, Gillette, Wyoming. [Abstract Only].  
 Curtin, et al., "CNT-reinforced ceramics and metals," Materials Today, 2004, vol. 7, pp. 44-49.  
 Flahaut, et al., "Carbon Nanotube-Metal-Oxide Nanocomposites: Microstructure, Electrical Conductivity and Mechanical Properties" Acta mater. 48 (2000), pp. 3803-3812.  
 Forsyth, et al.; "An Ionic Liquid Surface Treatment for Corrosion Protection of Magnesium Alloy AZ31"; Electrochem. Solid-State Lett. 2006 vol. 9, Issue 11, B52-B55/ 9(11); Abstract only; 1 page.  
 Galanty, et al. "Consolidation of metal powders during the extrusion process," Journal of Materials Processing Technology (2002), pp. 491-496.  
 Garfield, "Formation Damage Control Utilizing Composite-Bridge-Plug Technology for Monobore, Multizone Stimulation Operations," SPE 70004, 2001, Society of Petroleum Engineers Inc., This paper was prepared for presentation at the SPE Per.  
 Garfield, et al., "Maximizing Inflow Performance in Soft Sand Completions Using New One-trip Sand Control Liner completion Technology", SPE European Formation Damage Conference, May 25-27, 2005.  
 Goh, et al., "Development of novel carbon nanotube reinforced magnesium nanocomposites using the powder metallurgy technique", Nanotechnology 17 (2006) 7-12.  
 Han, et al., "Mechanical Properties of Nanostructured Materials", Rev. Adv. Mater. Sci. 9(2005) 1-16.  
 Hiermawan, et al., "Iron-manganese: new class of metallic degradable biomaterials prepared by powder metallurgy", Powder Metallurgy, vol. 51, No. 1, (2008), pp. 38-45.  
 Hjortstam, et al. "Can we achieve ultra-low resistivity in carbon nanotube-based metal composites," Applied Physics A (2004), vol. 78, Issue 8, pp. 1175-1179.  
 Hsiao, et al., "Baking Treatment Effect on Materials Characteristics and Electrochemical Behavior of anodic Film Formed on AZ91D Magnesium Alloy"; Corrosion Science; 49; pp. 781-793; (2007).  
 Hsiao, et al., "Effect of Heat Treatment on Anodization and Electrochemical Behavior of AZ91D Magnesium Alloy"; J. Mater. Res.; 20(10); pp. 2763-2771;(2005).  
 International Search Report and Written Opinion; International Application No. PCT/US2010/057763; International Filing Date: Nov. 23, 2010; dated Jul. 28, 2011; 10 pages.  
 International Search Report and Written Opinion; International Application No. PCT/US2010/059257; International Filing Date: Dec. 7, 2010; dated Jul. 27, 2011; 8 pages.  
 International Search Report and Written Opinion; International Application No. PCT/US2010/059259; International Filing Date: Dec. 7, 2010; dated Jun. 13, 2011; 8 pages.  
 International Search Report and Written Opinion; International Application No. PCT/US2010/059263; International Filing Date: Dec. 7, 2010; dated Jul. 8, 2011; 9 pages.  
 International Search Report and Written Opinion; International Application No. PCT/US2010/059265; International Filing Date: Dec. 7, 2010; dated Jun. 16, 2011; 8 pages.  
 International Search Report and Written Opinion; International Application No. PCT/US2010/059268; International Filing Date: Dec. 7, 2010; dated Jun. 17, 2011; 8 pages.  
 International Search Report and Written Opinion; International Application No. PCT/US2011/043036; International Filing Date: Jul. 6, 2011; dated Feb. 23, 2012; 9 pages.  
 International Search Report and Written Opinion; International Application No. PCT/US2011/047000; International Filing Date: Aug. 9, 2011; dated Dec. 26, 2011; 8 pages.  
 International Search Report and Written Opinion; International Application No. PCT/US2011/058099; International Filing Date: Oct. 27, 2011; dated May 11, 2012; 12 pages.  
 International Search Report and Written Opinion; International Application No. PCT/US2012/046231; International Filing Date: Jul. 11, 2012; dated Jan. 29, 2013; 9 pages.

(56)

## References Cited

## OTHER PUBLICATIONS

- International Search Report and Written Opinion; International Application No. PCT/US2012/049434; International Filing Date: Aug. 3, 2012; dated Feb. 1, 2013; 7 pages.
- International Search Report and Written Opinion; International Application No. PCT/US2012/053339; International Filing Date: Aug. 31, 2012; dated Feb. 15, 2013; 11 pages.
- International Search Report and Written Opinion; International Application No. PCT/US2012/053342; International Filing Date: Aug. 31, 2012; dated Feb. 19, 2013; 9 pages.
- International Search Report and Written Opinion; International Application No. PCT/US2012/053350; International Filing Date: Aug. 31, 2012; dated Feb. 25, 2013; 10 pages.
- International Search Report and Written Opinion; International Application No. PCT/US2012/071742; International Filing Date: Dec. 27, 2012; dated Apr. 22, 2013; 12 pages.
- Lavernia et al. "Cryomilled Nanostructured Materials: Processing and Properties", *Materials Science and Engineering A*, 493, (2008) pp. 207-214.
- Li, "Design of Abrasive Water Jet Perforation and Hydraulic Fracturing Tool," *Oil Field Equipment*, Mar. 2011.
- Maisano, "Cryomilling of Aluminum-Based and Magnesium-Based Metal Powders", Thesis, Virginia Tech, Jan. 13, 2006.
- Seyni, et al., "On the interest of using degradable fillers in co-ground composite materials", *Powder Technology* 190, (2009) pp. 176-184.
- Vahlas, et al., "Principles and Applications of CVD Powder Technology", *Materials Science and Engineering R* 53 (2006) pp. 1-72. "Optisleeve Sliding Sleeve", [online]; [retrieved on Jun. 25, 2010]; retrieved from the Internet [weatherfordcorp/WFT033159.pdf](http://weatherford.com/weatherford/groups/./weatherfordcorp/WFT033159.pdf).
- Baker Hughes, "Flow Control Systems," [online]; [retrieved on May 20, 2010]; retrieved from the Internet <http://www.bakerhughes.com/products-and-services/completions-and-productions/well-completions/packers-and-flow-control/flow-control-systems>.
- Bououdina, et al., "Comparative Study of Mechanical Alloying of (Mg+Al) and (Mg+Al+Ni) Mixtures for Hydrogen Storage", *J. Alloys. Compds.* 2002, 336, 222-231.
- Canadian Office Action for Canadian Application No. 2,783,241, dated Feb. 25, 2013, pp. 1-3.
- Canadian Office Action for Canadian Application No. 2,783,346, dated Feb. 21, 2013, pp. 1-4.
- Carrejo, et al., "Improving Flow Assurance in Multi-Zone Fracturing Treatments in Hydrocarbon Reservoirs with High Strength Corrodible Tripping Balls"; Society of Petroleum Engineers; SPE Paper No. 151613; Apr. 16, 2012; 5 pages.
- Coronado, "Development of an Internal Coiled Tubing Connector Utilizing Permanent Packer Technology"; Society of Petroleum Engineers, SPE Paper No. 46036; Apr. 15, 1998; 10 pages.
- Adams, et al.; "Thermal stabilities of aromatic acids as geothermal tracers", *Geothermics*, vol. 21, No. 3, 1992, pp. 323-339.
- Aviles et al, "Degradable Alternative to Risky Mill-Out Operations in Plug and Perf"; SPE-173695-MS; Society of Petroleum Engineers; SPE/ICOTA Coiled Tubing & Well Intervention Conference & Exhibition; Mar. 24-25, 2015; 10 Pages.
- Ayman, et al.; "Effect of Consolidation and Extrusion Temperatures on Tensile Properties of Hot Extruded ZK61 Magnesium Alloy Gas Atomized Powders via Spark Plasma Sintering", *Transactions of JWRI*, vol. 38 (2009), No. 2, pp. 1-5.
- Baker Hughes Incorporated. IN-Tallic Disintegrating Frac Balls. Houston: Baker Hughes Incorporated, 2011. Accessed Mar. 6, 2015.
- Baker Hughes, "Multistage", Oct. 31, 2011, [BakerHughes.com](http://BakerHughes.com); accessed Mar. 6, 2015.
- Bin et al., "Advances in Fluidization CVD Technology", East China University of Chemical Technology, China Academic Journal Electronic Publishing House, vol. 13, No. 4, Nov. 1992, pp. 360-365, English Abstract on p. 366.
- Canadian Office Action for Canadian Application No. 2,833,981, dated Sep. 23, 2014, pp. 1-2.
- Canadian Office Action for Canadian Application No. 2,834,794, dated Dec. 15, 2014, pp. 1-3.
- Canadian Office Action for Canadian Application No. 2,841,068, dated Jan. 23, 2015, pp. 1-3.
- Canadian Office Action for Canadian Application No. 2,841,078, dated Oct. 7, 2014, pp. 1-2.
- Canadian Office Action for Canadian Application No. 2,841,132, dated Mar. 11, 2015, pp. 1-4.
- Canadian Office Action for Canadian Application No. 2,841,184, dated Apr. 16, 2015, pp. 1-5.
- Canadian Office Action for Canadian Application No. 2,842,962, dated Mar. 19, 2015, pp. 1-6.
- Canadian Office Action for Canadian Application No. 2,843,011, dated Mar. 31, 2015, pp. 1-4.
- Canadian Office Action for Canadian Application No. 2,844,517, dated May 26, 2015, pp. 1-4.
- Canadian Office Action for Canadian Application No. 2,845,339, dated May 1, 2015, pp. 1-3.
- Canadian Office Action for Canadian Application No. 2,860,699, dated Jul. 16, 2015, pp. 1-4.
- Chinese Office Action; Chinese Application No. 201180052095.6; dated Mar. 18, 2015; pp. 1-19.
- Chinese Office Action; Chinese Application No. 201280036253.3; dated Apr. 22, 2015; 21 pages.
- Chinese Office Action; Chinese Application No. 201280036260.3; dated May 27, 2015; pp. 1-18.
- Danish Search Report and Opinion for Danish Application No. PA 2013 00060, dated Dec. 12, 2014, pp. 1-6.
- International Search Report and Written Opinion; International Application No. PCT/US2012/047163; International Filing Date: Jul. 18, 2012; dated Feb. 26, 2013; 12 pages.
- International Search Report and Written Opinion; International Application No. PCT/US2012/052836; International Filing Date: Aug. 29, 2012; dated Feb. 1, 2013; 9 pages.
- International Search Report and Written Opinion; International Application No. PCT/US2013/050475; International Filing Date: Jul. 15, 2013; dated Oct. 10, 2013; 12 pages.
- International Search Report and Written Opinion; International Application No. PCT/US2014/058997, International Filing Date: Oct. 3, 2014; dated Jan. 12, 2015; 12 pages.
- Lin et al., "Processing and Microstructure of Nano-Mo/Al<sub>2</sub>O<sub>3</sub> Composites from MOCVD and Fluidized Bed", *Nanostructured Materials*, Nov. 1999, vol. 11, No. 8, pp. 1361-1377.
- Rose, et al.; "The application of the polyaromatic sulfonates as tracers in geothermal reservoirs", *Geothermics* 30 (2001) pp. 617-640.
- Shigematsu, et al., "Surface Treatment of AZ91D Magnesium Alloy by Aluminum diffusion Coating", *Journal of Materials Science Letters* 19, 2000, pp. 473-475.
- Singh, et al., "Extended Homogeneity Range of Intermetallic Phases in Mechanically Alloyed Mg—Al Alloys", Elsevier Sciences Ltd., *Intermetallics* 11, 2003, pp. 373-376.
- Spencer et al., "Fluidized Bed Polymer Particle ALD Process for Producing HDPE/Alumina Nanocomposites", The 12th International Conference on Fluidization—New Horizons in Fluidization Engineering, vol. RP4 (2007).
- Stanley, et al.; "An Introduction to Ground-Water Tracers", Department of Hydrology and Water Resources, University of Arizona, Mar. 1985, pp. 1-219.
- Zemel, "Tracers in the Oil Field", University of Texas at Austin, Center for Petroleum and Geosystems, Jan. 1995, Chapters 1, 2, 3, 7.
- "Declaration of Karl T. Hartwig in Support of Petitioner Pursuant to 37 C.F.R. § 42.120", executed on Nov. 21, 2016 in support of U.S. Pat. No. 9,101,978, 51 pages.
- Xie, Guoqiang et al., "TEM Observation of Interfaces between Particles in Al—Mg Alloy Powder Compacts Prepared by Pulse Electric Current Sintering", *Materials Transactions*, 2002, pp. 2177-2180, vol. 43—No. 9.
- Callister, Jr., William D., *Materials Science and Engineering An Introduction*, Seventh Edition, 2006, pp. 111, 627, and G7.
- Canadian Office Action for Application No. 2860699; dated Oct. 7, 2015, 4 pages.

(56)

## References Cited

## OTHER PUBLICATIONS

- Chinese Office Action for Chinese Application No. 201280041320.0; dated Jun. 6, 2016, 14 pages.
- Chinese Office Action for Chinese Application No. 201380006291.9 dated Apr. 27, 2016, 25 pages.
- European Search Report for EP Application No. 12828903.0 dated Dec. 23, 2015.
- European Search Report for European Application No. 12820355.1-1353, dated Dec. 18, 2015, 9 pages.
- Schaffer, J.P. et al., *The Science and Design of Engineering Materials*, Second Edition, 1999, pp. 122, 123, 698, 699.
- International Search Report and Written Opinion, International Application No. PCT/US2016/041849, dated Oct. 26, 2016, Korean Intellectual Property Office; International Search Report 5 pages, Written Opinion 7 pages.
- International Search Report and Written Opinion; International Application No. PCT/US2015/066353; International Filing Date: Dec. 17, 2015; dated Apr. 1, 2016; 14 pages.
- Klar, Erhard, *ASM Handbook: International Metals Handbook—Powder Metallurgy*, vol. 7, 1997, pp. 14, 276, and 798.
- Reid, Gary Carl, "Literature evaluation of induced groundwater tracers, field tracer techniques, and hydrodynamic dispersion values in porous media", Thesis in Geosciences (Masters), Texas Tech University, Aug. 1981, 109 pages.
- Saravanan et al, "Mechanically Alloyed Carbon Nanotubes (CNT) Reinforced Nanocrystalline AA 4032: Synthesis and Characterization", *Journal of Minerals and Materials Characterization and Engineering*, vol. 9, No. 11 pp. 1027-1035 2010.
- "Baker Hughes Refines Expandable Tubular Technology with Abaqus and Isight", *Simulia Realistic Simulation News*, Jan./Feb. 2011, pp. 12-13.
- "Reactivity series", Wikipedia, [http://en.wikipedia.org/w/index.php?title=Reactivity\\_series&printable=yes](http://en.wikipedia.org/w/index.php?title=Reactivity_series&printable=yes) downloaded on May 18, 2014, 8 pages.
- Bakshi et al., "Carbon nanotube reinforced metal matrix composites—a review," *International Materials Reviews*; 2010, pp. 41-64, vol. 55, No. 1.
- Birbilis, et al., "Exploring Corrosion Protection of Mg via Ionic Liquid Pretreatment", *Surface & Coatings Technology*; 201, pp. 4496-4504, (2007).
- Canadian Office Action for Canadian Application No. 2,833,958, dated Sep. 23, 2014, pp. 1-2.
- Chinese Office Action for Chinese Application No. 2010800556135, dated Nov. 4, 2014, pp. 1-20.
- Chinese Office Action for Chinese Application No. 2011800124475, dated Jul. 3, 2014, 7 pages.
- Chinese Office Action for Chinese Application No. 201180052095.6, dated Jul. 21, 2014, pp. 1-32.
- Feng, et al., "Electroless Plating of Carbon Nanotubes with Silver" *Journal of Materials Science*, 39, (2004) pp. 3241-3243.
- International Search Report and Written Opinion; International Application No. PCT/US2012/038622; International Filing Date: May 18, 2012; dated Dec. 6, 2012; 12 pages.
- International Search Report and Written Opinion; International Application No. PCT/US2013/020046; International Filing Date: Jan. 3, 2013; dated Apr. 10, 2013; 7 pages.
- International Search Report and Written Opinion; International Application No. PCT/US2014/054720; International Filing Date: Sep. 9, 2014; dated Dec. 17, 2014; 10 pages.
- International Search Report for related PCT Application No. PCT/US2013/035258, dated Jul. 4, 2013, pp. 1-4.
- International Search Report for related PCT Application No. PCT/US2013/035261, dated Jul. 10, 2013, pp. 1-4.
- International Search Report for related PCT Application No. PCT/US2013/035262, dated Jul. 1, 2013, pp. 1-4.
- International Search Report for related PCT Application No. PCT/US2013/068062, dated Feb. 12, 2014, pp. 1-3.
- Lee, et al., "Effects of Ni addition on hydrogen storage properties of MgI7Al12 alloy", *Materials Chemistry and Physics*, 2011, 126, pp. 319-324.
- Li, et al., "Investigation of aluminium-based nanocomposites with ultra-high strength", *Materials Science and Engineering A*, 527, pp. 305-316, (2009).
- Liu, et al.; "Electroless Nickel Plating on AZ91 Mg Alloy Substrate"; *Surface & Coatings Technology*; 200; pp. 5087-5093; (2006).
- Mathis, "Sand Management: A Review of Approaches and Concerns", *Society of Petroleum Engineers, SPE Paper No. 82240, SPE European Formation Damage Conference*, The Hague, The Netherlands, May 13-14, 2003.
- Pardo, et al.; "Corrosion Behaviour of Magnesium/Aluminium Alloys in 3.5 wt% NaCl"; *Corrosion Science*; 50; pp. 823-834; (2008).
- Quik Drill Composite Frac Plug; Baker Hughes, Baker Oil Tools; Copyright 2002; 3 pages.
- Shi, et al.; "Influence of the Beta Phase on the Corrosion Performance of Anodised Coatings on Magnesium-Aluminium Alloys"; *Corrosion Science*; 47; pp. 2760-2777; (2005).
- Shimizu, et al., "Multi-walled carbon nanotube-reinforced magnesium alloy composites", *Scripta Materialia*, vol. 58, Issue 4, Feb. 2008, pp. 267-270.
- Shumbera, et al. "Improved Water Injector Performance in a Gulf of Mexico Deepwater Development Using an Openhole Frac Pack Completion and Downhole Filter System: Case History." *SPE Annual Technical Conference and Exhibition*, Oct. 5-8, 2003.
- Song, et al.; "Corrosion Mechanisms of Magnesium Alloys"; *Advanced Engineering Materials*; 1(1); pp. 11-33; (1999).
- Song, et al.; "Influence of Microstructure on the Corrosion of Diecast AZ91D"; *Corrosion Science*; 41; pp. 249-273; (1999).
- Song, et al.; "Understanding Magnesium Corrosion"; *Advanced Engineering Materials*; 5; No. 12; pp. 837-858; (2003).
- Sun, et al.; "Colloidal Processing of Carbon Nanotube/Alumina Composites" *Chem. Mater.* 2002, 14, pp. 5169-5172.
- Vickery, et al.; "New One-Trip Multi-Zone Frac Pack System with Positive Positioning." *European Petroleum conference*, Oct. 29-31, 2002, Aberdeen, UK. [Abstract Only].
- Zeng, et al. "Progress and Challenge for Magnesium Alloys as Biomaterials," *Advanced Engineering Materials*, vol. 10, Issue 8, Aug. 2008, pp. B3-B14.
- Zhang, et al.; "High Strength Nanostructured Materials and Their Oil Field Applications"; *Society of Petroleum Engineers; Conference Paper SPE 157092; SPE International Oilfield Nanotechnology Conference*, 2012; 6 pages.
- Zhang, et al.; "Metal Coating on Suspended Carbon Nanotubes and its Implication to Metal—Tube Interaction", *Chemical Physics Letters* 331 (2000) 35-41.
- "Declaration of Karl T. Hartwig in Support of Petitioner Pursuant to 37 C.F.R. § 42.120", executed on Nov. 21, 2016 in support of U.S. Pat. No. 8,573,295, 52 pages.
- German, Randall M., *Powder Metallurgy Science*, Second Edition, 1994, 102 pages.
- Petition for Inter Partes Review; Case No. IPR2017-00326; U.S. Pat. No. 9,101,978; dated Nov. 23, 2016; 46 pages.
- Petition for Inter Partes Review; Case No. IPR2017-00327; U.S. Pat. No. 8,573,295; dated Nov. 23, 2016; 53 pages.
- Zhu, et al., "The process of coating on ultrafine particles by surface hydrolysis reaction in a fluidized bed reactor", *Surface and Coatings Technology* 135 (2000) 14-17.
- Zhang, et al.; "Formation of metal nanowires on suspended single-walled carbon nanotubes" *Applied Physics Letter*, vol. 77, No. 19 (2000), pp. 3015-3017.
- Zhang, et al.; "Study on the Environmentally Friendly Anodizing of AZ91D Magnesium Alloy"; *Surface and Coatings Technology*; 161; pp. 36-43; (2002).
- Zhan, et al., "Single-wall carbon nanotubes as attractive toughening agents in alumina-based nanocomposites" *Nature Materials*, vol. 2., Jan. 2003, pp. 38-42.
- Xu, et al., "Nanostructured Material-Based Completion Tools Enhance Well Productivity"; *International Petroleum Technology Conference; Conference Paper IPTC 16538; International Petroleum Technology Conference 2013*; 4 pages.

(56)

## References Cited

## OTHER PUBLICATIONS

- Welch, et al., "Nonelastomeric Sliding Sleeve Maintains Long Term Integrity in HP/HT Application: Case Histories" [Abstract Only], SPE Eastern Regional Meeting, Oct. 23-25, 1996, Columbus, Ohio.
- Watarai, Trend of research and development for magnesium alloys-reducing the weight of structural materials in motor vehicles, (2006) Science and technology trends, Quaterly review No. 18, 84-97.
- Garfield, New One-Trip Sand-Control Completion System that Eliminates Formation Damage Resulting From conventional Perforating and Gravel-Pack Operations, SPE Annual Technical Conference and Exhibition, Oct. 9-12, 2005.
- Gray, et al., "Protective Coatings on Magnesium and Its Alloys—Critical Review", Journal of Alloys and Compounds 336 (2002), pp. 88-113.
- Hsiao, et al., "Anodization of AZ91D Magnesium Alloy in Silicate-Containing Electrolytes"; Surface & Coatings Technology; 199; pp. 127-134; (2005).
- Hsiao, et al., "Characterization of Anodic Films Formed on AZ91D Magnesium Alloy"; Surface & Coatings Technology; 190; pp. 299-308; (2005).
- Huo et al.; "Corrosion of AZ91D Magnesium Alloy with a Chemical Conversion Coating and Electroless Nickel Layer"; Corrosion Science: 46; pp. 1467-1477; (2004).
- International Search Report and Written Opinion; International Application No. PCT/US2011/058105; International Filing Date: Oct. 27, 2011; dated May 1, 2012; 8 pages.
- International Search Report and Written Opinion; International Application No. PCT/US2012/034973; International Filing Date: Apr. 25, 2012; dated Nov. 29, 2012; 8 pages.
- International Search Report and Written Opinion; International Application No. PCT/US2012/034978; International Filing Date: Apr. 25, 2012; dated Nov. 12, 2012; 9 pages.
- International Search Report and Written Opinion; International Application No. PCT/US2012/044866; International Filing Date: Jun. 29, 2012; dated Jan. 2, 2013; 9 pages.
- International Search Report and Written Opinion; International Application No. PCT/US2014/010862; International Filing Date: Jan. 9, 2014; dated Apr. 21, 2014; 9 pages.
- International Search Report; International Application No. PCT/US2012/044229, International Filing Date: Jun. 26, 2012; dated Jan. 30, 2013; 3 pages.
- Kuzumaki, et al.; "Mechanical Characteristics and Preparation of Carbon Nanotube Fiber-Reinforced Ti Composite", Advanced Engineering Materials, 2000, 2, No. 7.
- Liu, et al., "Calculated Phase Diagrams and the Corrosion of Die-Cast Mg—Al Alloys", Corrosion Science, 2009, 51, 606-619.
- Lunder et al.; "The Role of Mg17Al12 Phase in the Corrosion of Mg Alloy AZ91"; Corrosion; 45(9); pp. 741-748; (1989).
- Majumdar, et al., "Laser Surface Engineering of a Magnesium Alloy with Al +Al2O3", Surface and Coatings Technology 179 (2004) pp. 297-305.
- Murray, "Binary Alloy Phase Diagrams" Int. Met. Rev., 30(5) 1985 vol. 1, pp. 103-187.
- Nie, "Patents of Methods to Prepare Intermetallic Matrix Composites: A Review", Recent Patents on Materials Science 2008, vol. 1, pp. 232-240.
- Saravanan et al., "Mechanically Alloyed Carbon Nanotubes (CNT) Reinforced Nanocrystalline AA 4032: Synthesis and Characterization," Journal of Minerals & Materials Characterization & Engineering, vol. 9, No. 11, pp. 1027-1035, 2010.
- Shaw, "Benefits and Application of a Surface-Controlled Sliding Sleeve for Fracturing Operations"; Society of Petroleum Engineers, SPE Paper No. 147546; Oct. 30, 2011; 8 pages.
- Song, "Recent Progress in Corrosion and Protection of Magnesium Alloys"; Advanced Engineering Materials; 7(7); pp. 563-586; (2005).
- Song, et al.; "A Possible Biodegradable Magnesium Implant Material," Advanced Engineering Materials, vol. 9, Issue 4, Apr. 2007, pp. 298-302.
- Song, et al.; "Corrosion Behaviour of AZ21, AZ501 and AZ91 in Sodium Chloride"; Corrosion Science; 40(10); pp. 1769-1791; (1998).
- Triolo et al., "Resolving the Completion Engineer's Dilemma: Permanent or Retrievable Packer?"; Society of Petroleum Engineers, SPE Paper No. 76711; May 20, 2002; 16 pages.
- Vernon Constien et al., "Development of Reactive Coatings to Protect Sand-Control Screens", SPE 112494, Copyright 2008, Society of Petroleum Engineers, Presented at the 2008 SPE International Symposium and Exhibition on Formation Damage Control.
- Walters, et al.; "A Study of Jets from Unsintered-Powder Metal Lined Nonprecision Small-Caliber Shaped Charges", Army Research Laboratory, Aberdeen Proving Ground, MD 21005-5066; Feb. 2001.
- Wang, et al., "Contact-Damage-Resistant Ceramic/Single-Wall Carbon Nanotubes and Ceramic/Graphite Composites" Nature Materials, vol. 3, Aug. 2004, pp. 539-544.
- Watanabe, et al., "Superplastic Deformation Mechanism in Powder Metallurgy Magnesium Alloys and Composites", Acta mater. 49 (2001) pp. 2027-2037.
- Canadian Office Action for Canadian Application No. 2,841,068, dated Nov. 9, 2015, pp. 1-4.
- Chinese Office Action for Chinese Patent Application No. 201280041531.4 dated Aug. 31, 2015.
- European Search Report for EP Application No. 12827733.2 dated Jan. 21, 2015; 6 pages.
- European Search Report for EP Application No. 12827915.5 dated Dec. 23, 2015; 8 pages.
- Extended European Search Report for EP Application No. 12828379.3-1373, dated May 20, 2016, 8 pages.
- Extended European Search Report; EP Application No. 12822169.4-1605/2739812; dated Nov. 17, 2015; 9 pages.
- International Search Report and Written Opinion; International Application No. PCT/US2014/049347; International Filing Date: Aug. 1, 2014; dated Nov. 24, 2014; 11 pages.
- Office Action dated Mar. 23, 2016 in related EP Patent Application No. 12827733.2.
- Malaysian Search Report for Application No. PI 2012002545 dated May 31, 2016, 3 pages.
- Office Action dated Feb. 1, 2016 in related Canadian Patent Application No. 2,844,517, 4 pages.
- European Search Report for EP Application No. 10836533.9 dated Jul. 27, 2015.
- Australian Examination Report for Australian patent application No. 2012302067 dated Sep. 22, 2015.
- Australian Examination Report; Australian Application No. 2012287461; dated Jul. 13, 2015; 6 pages.
- Chinese Office Action for Chinese Application No. 201280036477.4, dated Nov. 4, 2015, pp. 1-15.
- Chinese Office Action; Chinese Application No. 201280020572.5; dated Oct. 10, 2015; 13 pages.
- Chuan-Jun et al., "Study on Corrosion Kinetics of Mg—Ni alloys", Journal of Kunming University of Science and Technology, vol. 34, No. 5, pp. 10-13, Oct. 2009.
- European Search Report for EP Application No. 10836538.8 dated Jul. 27, 2015.
- European Search Report for EP Application No. 10836540.4 dated Aug. 20, 2015.
- European Search Report for EP Application No. 10836539.6 dated Jul. 27, 2015.
- Tsipas et al. "Effect of High Energy Ball Milling on Titanium-Hydroxyapatite Powders" Powder Metallurgy, Maney Publishing, London, GB, vol. 46, No. 1, Mar. 2003 (Mar. 2003), pp. 73-77.
- Chinese Office Action; Chinese Application No. 201280041839.9; dated Feb. 10, 2015; pp. 1-37.
- Chinese Office Action; Chinese Application No. 201280041320.0; dated May 11, 2015; pp. 1-17.
- AP African Office Action for African Application No. AP/P/2014/007389, dated Oct. 6, 2016, 5 pages.
- EP Search Report, PCT/US2012049434; Application No. EP 12823958; dated Jun. 16, 2015; 9 pages.





FIG. 2



FIG. 3



## 1

MAGNESIUM ALLOY POWDER METAL  
COMPACTCROSS REFERENCE TO RELATED  
APPLICATIONS

This application is a divisional of and claims the benefit of an earlier filing date from U.S. application Ser. No. 13/220,824 filed Aug. 30, 2011, now U.S. Pat. No. 9,109,269, the entire disclosure of which is incorporated herein by reference.

## BACKGROUND

Oil and natural gas wells often utilize wellbore components or tools that, due to their function, are only required to have limited service lives that are considerably less than the service life of the well. After a component or tool service function is complete, it must be removed or disposed of in order to recover the original size of the fluid pathway for use, including hydrocarbon production, CO<sub>2</sub> sequestration, etc. Disposal of components or tools has conventionally been done by milling or drilling the component or tool out of the wellbore, which are generally time consuming and expensive operations.

In order to eliminate the need for milling or drilling operations, the removal of components or tools from the wellbore by dissolution or corrosion using various dissolvable or corrodible materials has been proposed. While these materials are useful, it is also very desirable that these materials be lightweight and have high strength, including a strength comparable to that of conventional engineering materials used to form wellbore components or tools, such as various grades of steel. Thus, the further improvement of dissolvable or corrodible materials to increase their strength, corrodibility and manufacturability is very desirable.

## SUMMARY

In an exemplary embodiment, a powder metal compact is disclosed. The powder metal compact includes a cellular nanomatrix comprising a nanomatrix material. The powder metal compact also includes a plurality of dispersed particles comprising a particle core material that comprises an Mg—Zr, Mg—Zn—Zr, Mg—Al—Zn—Mn, Mg—Zn—Cu—Mn or Mg—W alloy, or a combination thereof, dispersed in the cellular nanomatrix.

## BRIEF DESCRIPTION OF THE DRAWINGS

Referring now to the drawings wherein like elements are numbered alike in the several Figures:

FIG. 1 is a schematic illustration of an exemplary embodiment of a powder 10 and powder particles 12;

FIG. 2 is a schematic of illustration of an exemplary embodiment of the powder compact have an equiaxed configuration of dispersed particles as disclosed herein;

FIG. 3 is a schematic of illustration of an exemplary embodiment of the powder compact have a substantially elongated configuration of dispersed particles as disclosed herein;

FIG. 4 is a schematic of illustration of an exemplary embodiment of the powder compact have a substantially elongated configuration of the cellular nanomatrix and dispersed particles, wherein the cellular nanomatrix and dispersed particles are substantially continuous; and

## 2

FIG. 5 is a schematic of illustration of an exemplary embodiment of the powder compact have a substantially elongated configuration of the cellular nanomatrix and dispersed particles, wherein the cellular nanomatrix and dispersed particles are substantially discontinuous.

## DETAILED DESCRIPTION

Lightweight, high-strength magnesium alloy nanomatrix materials are disclosed. The magnesium alloys used to form these nanomatrix materials are high-strength magnesium alloys. Their strength may be enhanced through the incorporation of nanostructuring into the alloys. The strength of these alloys may also be improved by the incorporation of various strengthening subparticles and second particles. The magnesium alloy nanomatrix materials disclosed may also incorporate various microstructural features to control the alloy mechanical properties, such as the incorporation of a substantially elongated particle microstructure to enhance the alloy strength, or a multi-modal particle size in the alloy microstructural to enhance the fracture toughness, or a combination thereof to control both the strength, fracture toughness and other alloy properties.

The magnesium alloy nanomatrix materials disclosed herein may be used in all manner of applications and application environments, including use in various wellbore environments, to make various lightweight, high-strength articles, including downhole articles, particularly tools or other downhole components. In addition to their lightweight, high strength characteristics, these nanomatrix materials may be described as controlled electrolytic materials, which may be selectively and controllably disposable, degradable, dissolvable, corrodible or otherwise removable from the wellbore. Many other applications for use in both durable and disposable or degradable articles are possible. In one embodiment these lightweight, high-strength and selectively and controllably degradable materials include fully-dense, sintered powder compacts formed from coated powder materials that include various lightweight particle cores and core materials having various single layer and multilayer nanoscale coatings. In another embodiment, these materials include selectively and controllably degradable materials may include powder compacts that are not fully-dense or not sintered, or a combination thereof, formed from these coated powder materials.

Nanomatrix materials and methods of making these materials are described generally, for example, in U.S. patent application Ser. No. 12/633,682 filed on Dec. 8, 2009 and U.S. patent application Ser. No. 13/194,361 filed on Jul. 29, 2011, which are hereby incorporated herein by reference in their entirety. These lightweight, high-strength and selectively and controllably degradable materials may range from fully-dense, sintered powder compacts to precursor or green state (less than fully dense) compacts that may be sintered or unsintered. They are formed from coated powder materials that include various lightweight particle cores and core materials having various single layer and multilayer nanoscale coatings. These powder compacts are made from coated metallic powders that include various electrochemically-active (e.g., having relatively higher standard oxidation potentials) lightweight, high-strength particle cores and core materials, such as electrochemically active metals, that are dispersed within a cellular nanomatrix formed from the consolidation of the various nanoscale metallic coating layers of metallic coating materials, and are particularly useful in wellbore applications. The powder compacts may be made by any suitable powder compaction method,

including cold isostatic pressing (CIP), hot isostatic pressing (HIP), dynamic forging and extrusion, and combinations thereof. These powder compacts provide a unique and advantageous combination of mechanical strength properties, such as compression and shear strength, low density and selectable and controllable corrosion properties, particularly rapid and controlled dissolution in various wellbore fluids. The fluids may include any number of ionic fluids or highly polar fluids, such as those that contain various chlorides. Examples include fluids comprising potassium chloride (KCl), hydrochloric acid (HCl), calcium chloride (CaCl<sub>2</sub>), calcium bromide (CaBr<sub>2</sub>) or zinc bromide (ZnBr<sub>2</sub>). The disclosure of the '682 and '361 applications regarding the nature of the coated powders and methods of making and compacting the coated powders are generally applicable to provide the lightweight, high-strength magnesium alloy nanomatrix materials disclosed herein, and for brevity, are not repeated herein.

As illustrated in FIGS. 1 and 2, a powder 10 comprising powder particles 12, including a particle core 14 and core material 18 and metallic coating layer 16 and coating material 20, may be selected that is configured for compaction and sintering to provide a powder metal compact 200 that is lightweight (i.e., having a relatively low density), high-strength and is selectively and controllably removable from a wellbore in response to a change in a wellbore property, including being selectively and controllably dissolvable in an appropriate wellbore fluid, including various wellbore fluids as disclosed herein. The powder metal compact 200 includes a cellular nanomatrix 216 comprising a nanomatrix material 220 and a plurality of dispersed particles 214 comprising a particle core material 218 that comprises an Mg—Zr, Mg—Zn—Zr, Mg—Al—Zn—Mn, Mg—Zn—Cu—Mn or Mg—W alloy, or a combination thereof, dispersed in the cellular nanomatrix 216.

Dispersed particles 214 may comprise any of the materials described herein for particle cores 14, even though the chemical composition of dispersed particles 214 may be different due to diffusion effects as described herein. In an exemplary embodiment, dispersed particles 214 are formed from particle cores 14 comprising an Mg—Zr, Mg—Zn—Zr, Mg—Al—Zn—Mn, Mg—Zn—Cu—Mn or Mg—W alloy, or a combination thereof. In an exemplary embodiment, dispersed particles 214 include particle core material 218 comprising, in weight percent, about 6.0 to about 10.0 Al, about 0.3 to about 1.2 Zn, about 0.1 to about 0.6 Mn and the balance Mg and incidental impurities. In another exemplary embodiment, dispersed particles 214 include particle core material 218 comprising, in weight percent, about 0.5 to about 6.5 Zn, about 0.3 to about 0.75 Zr and the balance Mg and incidental impurities. Dispersed particles 214 and particle core material 218 may also include a rare earth element, or a combination of rare earth elements. As used herein, rare earth elements include Sc, Y, La, Ce, Pr, Nd or Er, or a combination of rare earth elements. Where present, a rare earth element or combination of rare earth elements may be present, by weight, in an amount of about 5 percent or less.

Dispersed particle 214 and particle core material 218 may also comprise a nanostructured material 215. In an exemplary embodiment, a nanostructured material 215 is a material having a grain size, or a subgrain or crystallite size, less than about 200 nm, and more particularly a grain size of about 10 nm to about 200 nm, and even more particularly an average grain size less than about 100 nm. The nanostructure may include high angle boundaries 227, which are usually used to define the grain size, or low angle boundaries 229

that may occur as substructure within a particular grain, which are sometimes used to define a crystallite size, or a combination thereof. The nanostructure may be formed in the particle core 14 used to form dispersed particle 214 by any suitable method, including deformation-induced nanostructure such as may be provided by ball milling a powder to provide particle cores 14, and more particularly by cryomilling (e.g., ball milling in ball milling media at a cryogenic temperature or in a cryogenic fluid, such as liquid nitrogen) a powder to provide the particle cores 14 used to form dispersed particles 214. The particle cores 14 may be formed as a nanostructured material 215 by any suitable method, such as, for example, by milling or cryomilling of prealloyed powder particles of the magnesium alloys described herein. The particle cores 14 may also be formed by mechanical alloying of pure metal powders of the desired amounts of the various alloy constituents. Mechanical alloying involves ball milling, including cryomilling, of these powder constituents to mechanically enfold and intermix the constituents and form particle cores 14. In addition to the creation of nanostructure as described above, ball milling, including cryomilling, may contribute to solid solution strengthening of the particle core 14 and core material 18, which in turn contribute to solid solution strengthening of dispersed particle 214 and particle core material 218. The solid solution strengthening may result from the ability to mechanically intermix a higher concentration of interstitial or substitutional solute atoms in the solid solution than is possible in accordance with the particular alloy constituent phase equilibria, thereby providing an obstacle to, or serving to restrict, the movement of dislocations within the particle, which in turn provides a strengthening mechanism in particle core 14 and dispersed particle 214. Particle core 14 may also be formed as a nanostructured material 215 by methods including inert gas condensation, chemical vapor condensation, pulse electron deposition, plasma synthesis, crystallization of amorphous solids, electrodeposition and severe plastic deformation, for example. The nanostructure also may include a high dislocation density, such as, for example, a dislocation density between about 10<sup>17</sup> m<sup>-2</sup> and 10<sup>18</sup> m<sup>-2</sup>, which may be two to three orders of magnitude higher than similar alloy materials deformed by traditional methods, such as cold rolling.

Dispersed particle 214 and particle core material 218 may also comprise a subparticle 222, and may preferably comprise a plurality of subparticles. Subparticle 222 provides a dispersion strengthening mechanism within dispersed particle 214 and provides an obstacle to, or serves to restrict, the movement of dislocations within the particle. Subparticle 222 may have any suitable size, and in an exemplary embodiment may have an average particle size of about 10 nm to about 1 micron, and more particularly may have an average particle size of about 50 nm to about 200 nm. Subparticle 222 may comprise any suitable form of subparticle, including an embedded subparticle 224, a precipitate 226 or a dispersoid 228. Embedded particle 224 may include any suitable embedded subparticle, including various hard subparticles. The embedded subparticle or plurality of embedded subparticles may include various metal, carbon, metal oxide, metal nitride, metal carbide, intermetallic compound or cermet particles, or a combination thereof. In an exemplary embodiment, hard particles may include Ni, Fe, Cu, Co, W, Al, Zn, Mn or Si, or an oxide, nitride, carbide, intermetallic compound or cermet comprising at least one of the foregoing, or a combination thereof. Embedded subparticle 224 may be embedded by any suitable method, including, for example, by ball milling or cryomilling hard par-

ticles together with the particle core material 18. A precipitate subparticle 226 may include any subparticle that may be precipitated within the dispersed particle 214, including precipitate subparticles 226 consistent with the phase equilibria of constituents of the magnesium alloy of interest and their relative amounts (e.g., a precipitation hardenable alloy), and including those that may be precipitated due to non-equilibrium conditions, such as may occur when an alloy constituent that has been forced into a solid solution of the alloy in an amount above its phase equilibrium limit, as is known to occur during mechanical alloying, is heated sufficiently to activate diffusion mechanisms that enable precipitation. Dispersoid subparticles 228 may include nanoscale particles or clusters of elements resulting from the manufacture of the particle cores 14, such as those associated with ball milling, including constituents of the milling media (e.g., balls) or the milling fluid (e.g., liquid nitrogen) or the surfaces of the particle cores 14 themselves (e.g., metallic oxides or nitrides). Dispersoid subparticles 228 may include, for example, Fe, Ni, Cr, Mn, N, O, C and H. The subparticles 222 may be located anywhere in conjunction with particle cores 14 and dispersed particles 214. In an exemplary embodiment, subparticles 222 may be disposed within or on the surface of dispersed particles 214, or a combination thereof, as illustrated in FIG. 1. In another exemplary embodiment, a plurality of subparticles 222 are disposed on the surface of the particle core 14 and dispersed particles 214 and may also comprise the nanomatrix material 216, as illustrated in FIG. 1.

Powder compact 200 includes a cellular nanomatrix 216 of a nanomatrix material 220 having a plurality of dispersed particles 214 dispersed throughout the cellular nanomatrix 216. The dispersed particles 214 may be equiaxed in a substantially continuous cellular nanomatrix 216, or may be substantially elongated as described herein and illustrated in FIG. 3. In the case where the dispersed particles 214 are substantially elongated, the dispersed particles 214 and the cellular nanomatrix 216 may be continuous or discontinuous, as illustrated in FIGS. 4 and 5, respectively. The substantially-continuous cellular nanomatrix 216 and nanomatrix material 220 formed of sintered metallic coating layers 16 is formed by the compaction and sintering of the plurality of metallic coating layers 16 of the plurality of powder particles 12, such as by CIP, HIP or dynamic forging. The chemical composition of nanomatrix material 220 may be different than that of coating material 20 due to diffusion effects associated with the sintering. Powder metal compact 200 also includes a plurality of dispersed particles 214 that comprise particle core material 218. Dispersed particle cores 214 and core material 218 correspond to and are formed from the plurality of particle cores 14 and core material 18 of the plurality of powder particles 12 as the metallic coating layers 16 are sintered together to form nanomatrix 216. The chemical composition of core material 218 may also be different than that of core material 18 due to diffusion effects associated with sintering.

As used herein, the use of the term cellular nanomatrix 216 does not connote the major constituent of the powder compact, but rather refers to the minority constituent or constituents, whether by weight or by volume. This is distinguished from most matrix composite materials where the matrix comprises the majority constituent by weight or volume. The use of the term substantially-continuous, cellular nanomatrix is intended to describe the extensive, regular, continuous and interconnected nature of the distribution of nanomatrix material 220 within powder compact 200. As used herein, "substantially-continuous" describes

the extension of the nanomatrix material throughout powder compact 200 such that it extends between and envelopes substantially all of the dispersed particles 214. Substantially-continuous is used to indicate that complete continuity and regular order of the nanomatrix around each dispersed particle 214 is not required. For example, defects in the coating layer 16 over particle core 14 on some powder particles 12 may cause bridging of the particle cores 14 during sintering of the powder compact 200, thereby causing localized discontinuities to result within the cellular nanomatrix 216, even though in the other portions of the powder compact the nanomatrix is substantially continuous and exhibits the structure described herein. In contrast, in the case of substantially elongated dispersed particles 214, such as those formed by extrusion, "substantially discontinuous" is used to indicate that incomplete continuity and disruption (e.g., cracking or separation) of the nanomatrix around each dispersed particle 214, such as may occur in a predetermined extrusion direction 622, or a direction transverse to this direction. As used herein, "cellular" is used to indicate that the nanomatrix defines a network of generally repeating, interconnected, compartments or cells of nanomatrix material 220 that encompass and also interconnect the dispersed particles 214. As used herein, "nanomatrix" is used to describe the size or scale of the matrix, particularly the thickness of the matrix between adjacent dispersed particles 214. The metallic coating layers that are sintered together to form the nanomatrix are themselves nanoscale thickness coating layers. Since the nanomatrix at most locations, other than the intersection of more than two dispersed particles 214, generally comprises the interdiffusion and bonding of two coating layers 16 from adjacent powder particles 12 having nanoscale thicknesses, the matrix formed also has a nanoscale thickness (e.g., approximately two times the coating layer thickness as described herein) and is thus described as a nanomatrix. Further, the use of the term dispersed particles 214 does not connote the minor constituent of powder compact 200, but rather refers to the majority constituent or constituents, whether by weight or by volume. The use of the term dispersed particle is intended to convey the discontinuous and discrete distribution of particle core material 218 within powder compact 200.

Powder compact 200 may have any desired shape or size, including that of a cylindrical billet, bar, sheet or other form that may be machined, formed or otherwise used to form useful articles of manufacture, including various wellbore tools and components. The pressing used to form precursor powder compact 100 and sintering and pressing processes used to form powder compact 200 and deform the powder particles 12, including particle cores 14 and coating layers 16, to provide the full density and desired macroscopic shape and size of powder compact 200 as well as its microstructure. The morphology (e.g. equiaxed or substantially elongated) of the dispersed particles 214 and cellular network 216 of particle layers results from sintering and deformation of the powder particles 12 as they are compacted and interdiffuse and deform to fill the interparticle spaces 15 (FIG. 1). The sintering temperatures and pressures may be selected to ensure that the density of powder compact 200 achieves substantially full theoretical density.

In an exemplary embodiment, dispersed particles 214 are formed from particle cores 14 dispersed in the cellular nanomatrix 216 of sintered metallic coating layers 16, and the nanomatrix 216 includes a solid-state metallurgical bond or bond layer, extending between the dispersed particles 214 throughout the cellular nanomatrix 216 that is formed at a sintering temperature ( $T_s$ ), where  $T_s$  is less than the melting

temperature of the coating ( $T_C$ ) and the melting temperature of the particle ( $T_P$ ). As indicated, solid-state metallurgical bond is formed in the solid state by solid-state interdiffusion between the coating layers 16 of adjacent powder particles 12 that are compressed into touching contact during the compaction and sintering processes used to form powder compact 200, as described herein. As such, sintered coating layers 16 of cellular nanomatrix 216 include a solid-state bond layer that has a thickness defined by the extent of the interdiffusion of the coating materials 20 of the coating layers 16, which will in turn be defined by the nature of the coating layers 16, including whether they are single or multilayer coating layers, whether they have been selected to promote or limit such interdiffusion, and other factors, as described herein, as well as the sintering and compaction conditions, including the sintering time, temperature and pressure used to form powder compact 200.

As nanomatrix 216 is formed, including the metallurgical bond and bond layer, the chemical composition or phase distribution, or both, of metallic coating layers 16 may change. Nanomatrix 216 also has a melting temperature ( $T_M$ ). As used herein,  $T_M$  includes the lowest temperature at which incipient melting or liquation or other forms of partial melting will occur within nanomatrix 216, regardless of whether nanomatrix material 220 comprises a pure metal, an alloy with multiple phases each having different melting temperatures or a composite, including a composite comprising a plurality of layers of various coating materials having different melting temperatures, or a combination thereof, or otherwise. As dispersed particles 214 and particle core materials 218 are formed in conjunction with nanomatrix 216, diffusion of constituents of metallic coating layers 16 into the particle cores 14 is also possible, which may result in changes in the chemical composition or phase distribution, or both, of particle cores 14. As a result, dispersed particles 214 and particle core materials 218 may have a melting temperature ( $T_{DP}$ ) that is different than  $T_P$ . As used herein,  $T_{DP}$  includes the lowest temperature at which incipient melting or liquation or other forms of partial melting will occur within dispersed particles 214, regardless of whether particle core material 218 comprise a pure metal, an alloy with multiple phases each having different melting temperatures or a composite, or otherwise. In one embodiment, powder compact 200 is formed at a sintering temperature ( $T_S$ ), where  $T_S$  is less than  $T_C$ ,  $T_P$ ,  $T_M$  and  $T_{DP}$ , and the sintering is performed entirely in the solid-state resulting in a solid-state bond layer. In another exemplary embodiment, powder compact 200 is formed at a sintering temperature ( $T_S$ ), where  $T_S$  is greater than or equal to one or more of  $T_C$ ,  $T_P$ ,  $T_M$  or  $T_{DP}$  and the sintering includes limited or partial melting within the powder compact 200 as described herein, and further may include liquid-state or liquid-phase sintering resulting in a bond layer that is at least partially melted and resolidified. In this embodiment, the combination of a predetermined  $T_S$  and a predetermined sintering time ( $t_S$ ) will be selected to preserve the desired microstructure that includes the cellular nanomatrix 216 and dispersed particles 214. For example, localized liquation or melting may be permitted to occur, for example, within all or a portion of nanomatrix 216 so long as the cellular nanomatrix 216/dispersed particle 214 morphology is preserved, such as by selecting particle cores 14,  $T_S$  and  $t_S$  that do not provide for complete melting of particle cores. Similarly, localized liquation may be permitted to occur, for example, within all or a portion of dispersed particles 214 so long as the cellular nanomatrix 216/dispersed particle 214 morphology is preserved, such as by selecting metallic

coating layers 16,  $T_S$  and  $t_S$  that do not provide for complete melting of the coating layer or layers 16. Melting of metallic coating layers 16 may, for example, occur during sintering along the metallic layer 16/particle core 14 interface, or along the interface between adjacent layers of multi-layer coating layers 16. It will be appreciated that combinations of  $T_S$  and  $t_S$  that exceed the predetermined values may result in other microstructures, such as an equilibrium melt/resolidification microstructure if, for example, both the nanomatrix 216 (i.e., combination of metallic coating layers 16) and dispersed particles 214 (i.e., the particle cores 14) are melted, thereby allowing rapid interdiffusion of these materials.

Particle cores 14 and dispersed particles 214 of powder compact 200 may have any suitable particle size. In an exemplary embodiment, the particle cores 14 may have a unimodal distribution and an average particle diameter or size of about 5  $\mu\text{m}$  to about 300  $\mu\text{m}$ , more particularly about 80  $\mu\text{m}$  to about 120  $\mu\text{m}$ , and even more particularly about 100  $\mu\text{m}$ . In another exemplary embodiment, which may include a multi-modal distribution of particle sizes, the particle cores 14 may have average particle diameters or size of about 50 nm to about 500  $\mu\text{m}$ , more particularly about 500 nm to about 300  $\mu\text{m}$ , and even more particularly about 5  $\mu\text{m}$  to about 300  $\mu\text{m}$ . In an exemplary embodiment, the particle cores 14 or the dispersed particles may have an average particle size of about 50 nm to about 500  $\mu\text{m}$ .

Dispersed particles 214 may have any suitable shape depending on the shape selected for particle cores 14 and powder particles 12, as well as the method used to sinter and compact powder 10. In an exemplary embodiment, powder particles 12 may be spheroidal or substantially spheroidal and dispersed particles 214 may include an equiaxed particle configuration as described herein. In another exemplary embodiment, dispersed particles may have a non-spherical shape. In yet another embodiment, the dispersed particles may be substantially elongated in a predetermined extrusion direction 622, such as may occur when using extrusion to form powder compact 200. As illustrated in FIG. 3-5, for example, a substantially elongated cellular nanomatrix 616 comprising a network of interconnected elongated cells of nanomatrix material 620 having a plurality of substantially elongated dispersed particle cores 614 of core material 618 disposed within the cells. Depending on the amount of deformation imparted to form elongated particles, the elongated coating layers and the nanomatrix 616 may be substantially continuous in the predetermined direction 622 as shown in FIG. 4, or substantially discontinuous as shown in FIG. 5.

The nature of the dispersion of dispersed particles 214 may be affected by the selection of the powder 10 or powders 10 used to make particle compact 200. In one exemplary embodiment, a powder 10 having a unimodal distribution of powder particle 12 sizes may be selected to form powder compact 200 and will produce a substantially homogeneous unimodal dispersion of particle sizes of dispersed particles 214 within cellular nanomatrix 216. In another exemplary embodiment, a plurality of powders 10 having a plurality of powder particles with particle cores 14 that have the same core materials 18 and different core sizes and the same coating material 20 may be selected and uniformly mixed as described herein to provide a powder 10 having a homogenous, multimodal distribution of powder particle 12 sizes, and may be used to form powder compact 200 having a homogeneous, multimodal dispersion of particle sizes of dispersed particles 214 within cellular nanomatrix 216. Similarly, in yet another exemplary embodiment,

ment, a plurality of powders **10** having a plurality of particle cores **14** that may have the same core materials **18** and different core sizes and the same coating material **20** may be selected and distributed in a non-uniform manner to provide a non-homogenous, multimodal distribution of powder particle sizes, and may be used to form powder compact **200** having a non-homogeneous, multimodal dispersion of particle sizes of dispersed particles **214** within cellular nanomatrix **216**. The selection of the distribution of particle core size may be used to determine, for example, the particle size and interparticle spacing of the dispersed particles **214** within the cellular nanomatrix **216** of powder compacts **200** made from powder **10**.

As illustrated generally in FIGS. 1 and 2, powder metal compact **200** may also be formed using coated metallic powder **10** and an additional or second powder **30**, as described herein. The use of an additional powder **30** provides a powder compact **200** that also includes a plurality of dispersed second particles **234**, as described herein, that are dispersed within the nanomatrix **216** and are also dispersed with respect to the dispersed particles **214**. Dispersed second particles **234** may be formed from coated or uncoated second powder particles **32**, as described herein. In an exemplary embodiment, coated second powder particles **32** may be coated with a coating layer **36** that is the same as coating layer **16** of powder particles **12**, such that coating layers **36** also contribute to the nanomatrix **216**. In another exemplary embodiment, the second powder particles **232** may be uncoated such that dispersed second particles **234** are embedded within nanomatrix **216**. As disclosed herein, powder **10** and additional powder **30** may be mixed to form a homogeneous dispersion of dispersed particles **214** and dispersed second particles **234** or to form a non-homogeneous dispersion of these particles. The dispersed second particles **234** may be formed from any suitable additional powder **30** that is different from powder **10**, either due to a compositional difference in the particle core **34**, or coating layer **36**, or both of them, and may include any of the materials disclosed herein for use as second powder **30** that are different from the powder **10** that is selected to form powder compact **200**. In an exemplary embodiment, dispersed second particles **234** may include Ni, Fe, Cu, Co, W, Al, Zn, Mn or Si, or an oxide, nitride, carbide, intermetallic compound or cermet comprising at least one of the foregoing, or a combination thereof.

Nanomatrix **216** is a substantially-continuous, cellular network of metallic coating layers **16** that are sintered to one another. The thickness of nanomatrix **216** will depend on the nature of the powder **10** or powders **10** used to form powder compact **200**, as well as the incorporation of any second powder **30**, particularly the thicknesses of the coating layers associated with these particles. In an exemplary embodiment, the thickness of nanomatrix **216** is substantially uniform throughout the microstructure of powder compact **200** and comprises about two times the thickness of the coating layers **16** of powder particles **12**. In another exemplary embodiment, the cellular network **216** has a substantially uniform average thickness between dispersed particles **214** of about 50 nm to about 5000 nm. Powder compacts **200** formed by extrusion may have much smaller thicknesses, and may become non-uniform and substantially discontinuous, as described herein.

Nanomatrix **216** is formed by sintering metallic coating layers **16** of adjacent particles to one another by interdiffusion and creation of bond layer as described herein. Metallic coating layers **16** may be single layer or multilayer structures, and they may be selected to promote or inhibit

diffusion, or both, within the layer or between the layers of metallic coating layer **16**, or between the metallic coating layer **16** and particle core **14**, or between the metallic coating layer **16** and the metallic coating layer **16** of an adjacent powder particle, the extent of interdiffusion of metallic coating layers **16** during sintering may be limited or extensive depending on the coating thicknesses, coating material or materials selected, the sintering conditions and other factors. Given the potential complexity of the interdiffusion and interaction of the constituents, description of the resulting chemical composition of nanomatrix **216** and nanomatrix material **220** may be simply understood to be a combination of the constituents of coating layers **16** that may also include one or more constituents of dispersed particles **214**, depending on the extent of interdiffusion, if any, that occurs between the dispersed particles **214** and the nanomatrix **216**. Similarly, the chemical composition of dispersed particles **214** and particle core material **218** may be simply understood to be a combination of the constituents of particle core **14** that may also include one or more constituents of nanomatrix **216** and nanomatrix material **220**, depending on the extent of interdiffusion, if any, that occurs between the dispersed particles **214** and the nanomatrix **216**.

In an exemplary embodiment, the nanomatrix material **220** has a chemical composition and the particle core material **218** has a chemical composition that is different from that of nanomatrix material **220**, and the differences in the chemical compositions may be configured to provide a selectable and controllable dissolution rate, including a selectable transition from a very low dissolution rate to a very rapid dissolution rate, in response to a controlled change in a property or condition of the wellbore proximate the compact **200**, including a property change in a wellbore fluid that is in contact with the powder compact **200**, as described herein. Nanomatrix **216** may be formed from powder particles **12** having single layer and multilayer coating layers **16**. This design flexibility provides a large number of material combinations, particularly in the case of multilayer coating layers **16**, that can be utilized to tailor the cellular nanomatrix **216** and composition of nanomatrix material **220** by controlling the interaction of the coating layer constituents, both within a given layer, as well as between a coating layer **16** and the particle core **14** with which it is associated or a coating layer **16** of an adjacent powder particle **12**.

In an exemplary embodiment, nanomatrix **216** may comprise a nanomatrix material **220** comprising Ni, Fe, Cu, Co, W, Al, Zn, Mn, Mg or Si, or an alloy thereof, or an oxide, nitride, carbide, intermetallic compound or cermet comprising at least one of the foregoing, or a combination thereof.

The powder metal compacts **200** disclosed herein may be configured to provide selectively and controllably disposable, degradable, dissolvable, corrodible or otherwise removable from a wellbore using a predetermined wellbore fluid, including those described herein. These materials may be configured to provide a rate of corrosion up to about 500 mg/cm<sup>2</sup>/hr, and more particularly a rate of corrosion of about 0.5 to about 50 mg/cm<sup>2</sup>/hr. These powder compacts **200** may also be configured to provide high strength, including an ultimate compressive strength up to about 85 ksi, and more particularly from about 40 ksi to about 70 ksi.

The terms “a” and “an” herein do not denote a limitation of quantity, but rather denote the presence of at least one of the referenced items. The modifier “about” used in connection with a quantity is inclusive of the stated value and has the meaning dictated by the context (e.g., includes the degree of error associated with measurement of the particu-

## 11

lar quantity). Furthermore, unless otherwise limited all ranges disclosed herein are inclusive and combinable (e.g., ranges of “up to about 25 weight percent (wt. %), more particularly about 5 wt. % to about 20 wt. % and even more particularly about 10 wt. % to about 15 wt. %” are inclusive of the endpoints and all intermediate values of the ranges, e.g., “about 5 wt. % to about 25 wt. %, about 5 wt. % to about 15 wt. %”, etc.). The use of “about” in conjunction with a listing of constituents of an alloy composition is applied to all of the listed constituents, and in conjunction with a range to both endpoints of the range. Finally, unless defined otherwise, technical and scientific terms used herein have the same meaning as is commonly understood by one of skill in the art to which this invention belongs. The suffix “(s)” as used herein is intended to include both the singular and the plural of the term that it modifies, thereby including one or more of that term (e.g., the metal(s) includes one or more metals). Reference throughout the specification to “one embodiment”, “another embodiment”, “an embodiment”, and so forth, means that a particular element (e.g., feature, structure, and/or characteristic) described in connection with the embodiment is included in at least one embodiment described herein, and may or may not be present in other embodiments.

It is to be understood that the use of “comprising” in conjunction with the alloy compositions described herein specifically discloses and includes the embodiments wherein the alloy compositions “consist essentially of” the named components (i.e., contain the named components and no other components that significantly adversely affect the basic and novel features disclosed), and embodiments wherein the alloy compositions “consist of” the named components (i.e., contain only the named components except for contaminants which are naturally and inevitably present in each of the named components).

While one or more embodiments have been shown and described, modifications and substitutions may be made thereto without departing from the spirit and scope of the invention. Accordingly, it is to be understood that the present invention has been described by way of illustrations and not limitation.

The invention claimed is:

1. A powder metal compact, comprising:

a cellular nanomatrix comprising a nanomatrix material comprising Ni, Co, or an intermetallic compound comprising Ni or Co; a plurality of dispersed particles comprising a particle core material that comprises an Mg—Zr, Mg—Zn—Zr, Mg—Al—Zn—Mn, Mg—Zn—Cu—Mn or Mg—W alloy, or a combination thereof, dispersed in the cellular nanomatrix.

2. The powder metal compact of claim 1, wherein the particle core material comprises, in weight percent, about 0.5 to about 6.5 Zn, about 0.3 to about 0.75 Zr and the balance Mg and incidental impurities.

3. The powder metal compact of claim 1, wherein the particle core material comprises, in weight percent, about 6.0 to about 10.0 Al, about 0.3 to about 1.2 Zn, about 0.1 to about 0.6 Mn and the balance Mg and incidental impurities.

4. The powder metal compact of claim 1, wherein the particle core material or the nanomatrix material, or a combination thereof, comprises a nanostructured material.

5. The powder metal compact of claim 4, wherein the nanostructured material has a grain size less than about 200 nm.

## 12

6. The powder metal compact of claim 5, wherein the nanostructured material has a grain size of about 10 nm to about 200 nm.

7. The powder metal compact of claim 4, wherein the nanostructured material has an average grain size less than about 100 nm.

8. The powder metal compact of claim 1, wherein the dispersed particle further comprises a subparticle.

9. The powder metal compact of claim 8, wherein the subparticle has an average particle size of about 10 nm to about 1 micron.

10. The powder metal compact of claim 8, wherein the subparticle comprises a preformed subparticle, a precipitate or a dispersoid.

11. The powder metal compact of claim 8, wherein the subparticle is disposed within or on the surface of the dispersed particle, or a combination thereof.

12. The powder metal compact of claim 11, wherein the subparticle is disposed on the surface of the dispersed particle and also comprises the nanomatrix material.

13. The powder metal compact of claim 1, wherein the dispersed particles have an average particle size of about 50 nm to about 500  $\mu$ m.

14. The powder metal compact of claim 1, wherein the dispersed particles comprise a multi-modal distribution of particle sizes within the cellular nanomatrix.

15. The powder metal compact of claim 1, wherein the particle core material further comprises a rare earth element.

16. The powder metal compact of claim 1, wherein the dispersed particles have an equiaxed particle shape and the nanomatrix is substantially continuous.

17. The powder metal compact of claim 1, wherein the nanomatrix and the dispersed particles are substantially elongated in a predetermined direction.

18. The powder metal compact of claim 17, wherein the nanomatrix is substantially continuous.

19. The powder metal compact of claim 17, wherein the nanomatrix and the dispersed particles are discontinuous.

20. The powder metal compact of claim 1, further comprising a plurality of dispersed second particles, wherein the dispersed second particles are also dispersed within the cellular nanomatrix and with respect to the dispersed particles.

21. The powder metal compact of claim 20, wherein the dispersed second particles comprise a metal, carbon, metal oxide, metal nitride, metal carbide, intermetallic compound or cermet, or a combination thereof.

22. The powder metal compact of claim 21, wherein the dispersed second particles comprise Ni, Fe, Cu, Co, Mg, W, Al, Zn, Mn or Si, or an oxide, nitride, carbide, intermetallic compound or cermet comprising at least one of the foregoing, or a combination thereof.

23. The powder metal compact of claim 1, wherein the nanomatrix material comprises a constituent of a milling medium or a milling fluid.

24. The powder metal compact of claim 1, wherein the nanomatrix material comprises a multilayer material.

25. The powder metal compact of claim 1, wherein the nanomatrix material has a chemical composition and the particle core material has a chemical composition that is different than the chemical composition of the nanomatrix material.

26. The powder metal compact of claim 1, wherein the cellular nanomatrix has an average thickness of about 50 nm to about 5000 nm.

**27.** The powder metal compact of claim **1**, further comprising a bond layer extending throughout the cellular nano-matrix between the dispersed particles.

**28.** The powder metal compact of claim **27**, wherein the bond layer comprises a substantially solid state bond layer. 5

\* \* \* \* \*